



US007785757B2

(12) **United States Patent**  
**Yanus et al.**

(10) **Patent No.:** **US 7,785,757 B2**  
(45) **Date of Patent:** **\*Aug. 31, 2010**

(54) **OVERCOATED PHOTOCONDUCTORS WITH THIOPHOSPHATE CONTAINING PHOTOGENERATING LAYER**

(75) Inventors: **John F Yanus**, Webster, NY (US); **Jin Wu**, Webster, NY (US); **Kenny-Tuan Dinh**, Webster, NY (US); **Michael A. Morgan**, Fairport, NY (US); **Anthony M. Horgan**, Pittsford, NY (US); **Kathleen M. Carmichael**, Williamson, NY (US)

(73) Assignee: **Xerox Corporation**, Norwalk, CT (US)

(\*) Notice: Subject to any disclaimer, the term of this patent is extended or adjusted under 35 U.S.C. 154(b) by 905 days.

This patent is subject to a terminal disclaimer.

(21) Appl. No.: **11/593,662**

(22) Filed: **Nov. 7, 2006**

(65) **Prior Publication Data**

US 2008/0107983 A1 May 8, 2008

(51) **Int. Cl.**

**G03G 15/02** (2006.01)

(52) **U.S. Cl.** ..... **430/58.75**; 430/59.1; 430/66; 430/132

(58) **Field of Classification Search** ..... **430/58.75**, 430/59.1, 66, 132

See application file for complete search history.

(56) **References Cited**

U.S. PATENT DOCUMENTS

|             |         |                  |
|-------------|---------|------------------|
| 3,121,006 A | 2/1964  | Middleton et al. |
| 4,265,990 A | 5/1981  | Stolka et al.    |
| 4,464,450 A | 8/1984  | Teuscher         |
| 4,587,189 A | 5/1986  | Hor et al.       |
| 4,921,769 A | 5/1990  | Yuh et al.       |
| 4,921,773 A | 5/1990  | Melnyk et al.    |
| 5,473,064 A | 12/1995 | Mayo et al.      |

|                |        |                          |
|----------------|--------|--------------------------|
| 5,482,811 A    | 1/1996 | Keoshkerian et al.       |
| 5,521,306 A    | 5/1996 | Burt et al.              |
| 5,607,896 A *  | 3/1997 | Hutt ..... 503/227       |
| 6,913,863 B2   | 7/2005 | Wu et al.                |
| 7,037,631 B2   | 5/2006 | Wu et al.                |
| 7,498,108 B2 * | 3/2009 | Wu et al. ..... 430/59.1 |
| 7,541,122 B2 * | 6/2009 | Wu et al. ..... 430/58.2 |
| 7,572,561 B2 * | 8/2009 | Dinh et al. ..... 430/66 |

OTHER PUBLICATIONS

Jin Wu et al., U.S. Appl. No. 11/485,645 on Silanol Containing Photoconductors, filed Jun. 12, 2006.

Jin Wu et al., U.S. Appl. No. 11/485,550 on Silanol Containing Photoconductors, filed Jun. 12, 2006.

Jin Wu et al., U.S. Appl. No. 11/453,392 on Ether Phosphate Containing Photoconductors, filed Jun. 15, 2006.

Jin Wu et al., U.S. Appl. No. 11/453,621 on Ether Phosphate Containing Photoconductors, filed Jun. 15, 2006.

Jin Wu et al., U.S. Appl. No. 11/453,621 on Polyphenyl Ether Containing Photoconductors, filed Jun. 15, 2006.

Jin Wu et al., U.S. Appl. No. 11/453,379 on Polyphenyl Ether Phosphate Containing Photoconductors, filed Jun. 15, 2006.

Jin Wu et al., U.S. Appl. No. 11/453,742 on Polyphenyl Ether Phosphate Containing Photoconductors, filed Jun. 15, 2006.

Jin Wu et al., U.S. Appl. No. 11/453,740 on Polyphenyl Thioether Phosphate Containing Photoconductors, filed Jun. 15, 2006.

Jin Wu et al., U.S. Appl. No. 11/453,607 on Polyphenyl Thioether Phosphate Containing Photoconductors, filed Jun. 15, 2006.

Jin Wu et al., U.S. Appl. No. 11/453,739 on Polyphenyl Thioether Phosphate Containing Photoconductors, filed Jun. 15, 2006.

Jin Wu et al., U.S. Appl. No. 11/453,613 on Thiophosphate Containing Photoconductors, filed Jun. 15, 2006.

Jin Wu et al., U.S. Appl. No. 11/453,743 on Thiophosphate Containing Photoconductors, filed Jun. 15, 2006.

Jin Wu et al., U.S. Appl. No. 11/453,489 on Thiophosphate Containing Photoconductors, filed Jun. 15, 2006.

\* cited by examiner

*Primary Examiner*—Thorl Chea

(74) *Attorney, Agent, or Firm*—E. O. Palazzo

(57) **ABSTRACT**

A photoconductor containing a thiophosphate photogenerating layer, and at least one charge transport layer, and a top polymeric overcoating layer in contact with and contiguous to a charge transport layer.

**36 Claims, No Drawings**

## 1

OVERCOATED PHOTOCONDUCTORS WITH  
THIOPHOSPHATE CONTAINING  
PHOTOGENERATING LAYERCROSS REFERENCE TO RELATED  
APPLICATIONS

The disclosures of each of the following copending applications are totally incorporated herein by reference.

U.S. application Ser. No. 11/593,657, filed Nov. 7, 2006, 10 U.S. Publication No. 20080107984, on Overcoated Photoconductors with Thiophosphate Containing Charge Transport Layers, by John F. Yanus et al.

U.S. application Ser. No. 11/593,875, filed Nov. 7, 2006, 15 U.S. Publication No. 20080107985, on Silanol Containing Overcoated Photoconductors, by John F. Yanus et al.

U.S. application Ser. No. 11/593,656, filed Nov. 7, 2006, 20 U.S. Publication No. 20080107979, on Silanol Containing charge Transport Overcoated Photoconductors, by John F. Yanus et al.

In U.S. application Ser. No. 11/485,645, now U.S. Pat. No. 25 7,560,206, filed Jun. 12, 2006 by Jin Wu et al., there is illustrated an imaging member comprising an optional supporting substrate, a photogenerating layer containing a silanol, and at least one charge transport layer comprised of at least one charge transport component.

In U.S. application Ser. No. 11/485,550, now U.S. Pat. No. 30 7,541,122, filed Jun. 12, 2006 by Jin Wu et al., there is illustrated an imaging member comprising an optional supporting substrate, a photogenerating layer, and at least one charge transport layer comprised of at least one charge transport component, and at least one silanol.

U.S. application Ser. No. 11/453,392, now U.S. Pat. No. 35 7,479,358, filed Jun. 15, 2006 on Ether Phosphate Containing Photoconductors, by Jin Wu et al.

U.S. application Ser. No. 11/453,621, now U.S. Pat. No. 40 7,445,876, filed Jun. 15, 2006 on Ether Phosphate Containing Photoconductors, by Jin Wu et al.

U.S. application Ser. No. 11/453,622, now U.S. Pat. No. 45 7,459,250, filed Jun. 15, 2006 on Polyphenyl Ether Containing Photoconductors, by Jin Wu et al.

U.S. application Ser. No. 11/453,379, now U.S. Pat. No. 50 7,507,510, filed Jun. 15, 2006 on Polyphenyl Ether Phosphate Containing Photoconductors, by Jin Wu et al.

U.S. application Ser. No. 11/453,742, now U.S. Pat. No. 55 7,452,643, filed Jun. 15, 2006 on Polyphenyl Ether Phosphate Containing Photoconductors, by Jin Wu et al.

U.S. application Ser. No. 11/453,740, now U.S. Pat. No. 60 7,476,478, filed Jun. 15, 2006 on Polyphenyl Thioether Containing Photoconductors, by Jin Wu et al.

U.S. application Ser. No. 11/453,607, now U.S. Pat. No. 65 7,462,432, filed Jun. 15, 2006 on Polyphenyl Thioether Phosphate Containing Photoconductors, by Jin Wu et al.

U.S. application Ser. No. 11/453,739, now U.S. Pat. No. 70 7,468,229, filed Jun. 15, 2006 on Polyphenyl Thioether Phosphate Containing Photoconductors, by Jin Wu et al.

U.S. application Ser. No. 11/453,613, now U.S. Pat. No. 75 7,476,477, filed Jun. 15, 2006 on Thiophosphate Containing Photoconductors, by Jin Wu et al.

U.S. application Ser. No. 11/453,743, now U.S. Pat. No. 80 7,498,108, filed Jun. 15, 2006 on Thiophosphate Containing Photoconductors, by Jin Wu et al.

U.S. application Ser. No. 11/453,489, now U.S. Pat. No. 85 7,491,480, filed Jun. 15, 2006 on Thiophosphate Containing Photoconductors, by Jin Wu et al.

A number of the components and amounts thereof of the above copending applications, such as the supporting sub-

## 2

strates, resin binders, photogenerating layer components, antioxidants, charge transport components, silanols, dialkyldithiophosphates, hole blocking layer components, adhesive layers, and the like, may be selected for the members of the 5 present disclosure in embodiments thereof.

## BACKGROUND

This disclosure is generally directed to layered imaging members, photoreceptors, photoconductors, and the like. More specifically, the present disclosure is directed to multi-layered flexible, belt imaging members, or devices comprised of an optional supporting medium like a substrate, a thiophosphate containing photogenerating layer, or a thiophosphate, such as a zinc dialkyldithiophosphate (ZDDP), containing charge transport layer, including a plurality of charge transport layers, such as a first charge transport layer and a second charge transport layer, an optional adhesive layer, an optional hole blocking or undercoat layer, and an overcoating layer, 20 and optionally wherein at least one of the charge transport layers contains at least one charge transport component, a polymer or resin binder, a dialkyldithiophosphate, and an optional antioxidant. Moreover, at least one of the charge transport layers can be free of a dialkyldithiophosphate; and in embodiments, the photogenerating layer contains a dialkyldithiophosphate, and the charge transport layers are free of a dialkyldithiophosphate; and in embodiments, the charge transport layer contains a dialkylthiophosphate, and the photogenerating layer is free, that is this layer does not contain a dialkyldithiophosphate.

The photoreceptors illustrated herein, in embodiments, have excellent wear resistance, extended lifetimes, elimination or minimization of imaging member scratches, and which scratches can result in undesirable print failures where, 30 for example, the scratches are visible on the final prints generated. Additionally, in embodiments the imaging members disclosed herein possess excellent, and in a number of instances low  $V_r$  (residual potential), and allow the substantial prevention of  $V_r$  cycle up when appropriate; high sensitivity; low acceptable image ghosting characteristics; low background and/or minimal charge deficient spots (CDS); and desirable toner cleanability. More specifically, there is illustrated herein in embodiments the incorporation of suitable dialkyldithiophosphates in an imaging member, which 35 dialkyldithiophosphates can be included in at least one charge transport layer, the photogenerating layer, or in both the at least one charge transport layer and the photogenerating layer. At least one in embodiments refers, for example, to one, to from 1 to about 10, to from 2 to about 7; to from 2 to about 4, to 2, and the like. Moreover, the dialkyldithiophosphates, 40 which in embodiments are transparent and substantially soluble in the charge transport layers solution, can be added to the at least one of the charge transport layers, that is for example, instead of being dissolved in the charge transport 45 layer solution, the dialkyldithiophosphates can be added to the charge transport as a dopant, and more specifically, the dialkyldithiophosphates can be added to the top charge transport layer. Similarly, the dialkyldithiophosphates can be included in the photogenerating layer dispersion prior to the 50 deposition of this layer on the substrate.

Also included within the scope of the present disclosure are methods of imaging and printing with the photoresponsive or photoconductor devices illustrated herein. These methods generally involve the formation of an electrostatic latent 55 image on the imaging member, followed by developing the image with a toner composition comprised, for example, of thermoplastic resin, colorant, such as pigment, charge addi-

tive, and surface additive, reference U.S. Pat. Nos. 4,560,635; 4,298,697 and 4,338,390, the disclosures of which are totally incorporated herein by reference, subsequently transferring the image to a suitable substrate, and permanently affixing the image thereto. In those environments wherein the device is to be used in a printing mode, the imaging method involves the same operation with the exception that exposure can be accomplished with a laser device or image bar. More specifically, flexible belts disclosed herein can be selected for the Xerox Corporation iGEN3® machines that generate with some versions over 100 copies per minute. Processes of imaging, especially xerographic imaging and printing, including digital, and/or color printing, are thus encompassed by the present disclosure. The imaging members are in embodiments sensitive in the wavelength region of, for example, from about 400 to about 900 nanometers, and in particular from about 650 to about 850 nanometers, thus diode lasers can be selected as the light source. Moreover, the imaging members of this disclosure are useful in high resolution color xerographic applications, particularly high speed color copying and printing processes.

## REFERENCES

There is illustrated in U.S. Pat. No. 7,037,631, the disclosure of which is totally incorporated herein by reference, a photoconductive imaging member comprised of a supporting substrate, a hole blocking layer thereover, a crosslinked photogenerating layer and a charge transport layer, and wherein the photogenerating layer is comprised of a photogenerating component and a vinyl chloride, allyl glycidyl ether, hydroxy containing polymer.

There is illustrated in U.S. Pat. No. 6,913,863, the disclosure of which is totally incorporated herein by reference, a photoconductive imaging member comprised of a hole blocking layer, a photogenerating layer, and a charge transport layer, and wherein the hole blocking layer is comprised of a metal oxide; and a mixture of a phenolic compound and a phenolic resin wherein the phenolic compound contains at least two phenolic groups.

Layered photoresponsive imaging members have been described in numerous U.S. patents, such as U.S. Pat. No. 4,265,990, the disclosure of which is totally incorporated herein by reference, wherein there is illustrated an imaging member comprised of a photogenerating layer, and an aryl amine hole transport layer. Examples of photogenerating layer components include trigonal selenium, metal phthalocyanines, vanadyl phthalocyanines, and metal free phthalocyanines. Additionally, there is described in U.S. Pat. No. 3,121,006, the disclosure of which is totally incorporated herein by reference, a composite xerographic photoconductive member comprised of finely divided particles of a photoconductive inorganic compound and an amine hole transport dispersed in an electrically insulating organic resin binder.

Further, in U.S. Pat. No. 4,555,463, the disclosure of which is totally incorporated herein by reference, there is illustrated a layered imaging member with a chloroindium phthalocyanine photogenerating layer. In U.S. Pat. No. 4,587,189, the disclosure of which is totally incorporated herein by reference, there is illustrated a layered imaging member with, for example, a perylene, pigment photogenerating component. Both of the aforementioned patents disclose an aryl amine component, such as N,N'-diphenyl-N,N'-bis(3-methylphenyl)-1,1'-biphenyl-4,4'-diamine dispersed in a polycarbonate binder as a hole transport layer. The above components, such as the photogenerating compounds and the aryl amine charge

transport, can be selected for the imaging members of the present disclosure in embodiments thereof.

In U.S. Pat. No. 4,921,769, the disclosure of which is totally incorporated herein by reference, there are illustrated photoconductive imaging members with blocking layers of certain polyurethanes.

Illustrated in U.S. Pat. No. 5,521,306, the disclosure of which is totally incorporated herein by reference, is a process for the preparation of Type V hydroxygallium phthalocyanine comprising the in situ formation of an alkoxy-bridged gallium phthalocyanine dimer, hydrolyzing the dimer to hydroxygallium phthalocyanine, and subsequently converting the hydroxygallium phthalocyanine product to Type V hydroxygallium phthalocyanine.

Illustrated in U.S. Pat. No. 5,482,811, the disclosure of which is totally incorporated herein by reference, is a process for the preparation of hydroxygallium phthalocyanine photo-generating pigments which comprises hydrolyzing a gallium phthalocyanine precursor pigment by dissolving the hydroxygallium phthalocyanine in a strong acid, and then reprecipitating the resulting dissolved pigment in basic aqueous media; removing any ionic species formed by washing with water; concentrating the resulting aqueous slurry comprised of water and hydroxygallium phthalocyanine to a wet cake; removing water from said slurry by azeotropic distillation with an organic solvent, and subjecting said resulting pigment slurry to mixing with the addition of a second solvent to cause the formation of said hydroxygallium phthalocyanine polymorphs.

Also, in U.S. Pat. No. 5,473,064, the disclosure of which is totally incorporated herein by reference, there is illustrated a process for the preparation of photogenerating pigments of hydroxygallium phthalocyanine Type V essentially free of chlorine, whereby a pigment precursor Type I chlorogallium phthalocyanine is prepared by reaction of gallium chloride in a solvent, such as N-methylpyrrolidone, present in an amount of from about 10 parts to about 100 parts, and preferably about 19 parts with 1,3-diiminoisoindolene (DI<sup>3</sup>) in an amount of from about 1 part to about 10 parts, and preferably about 4 parts of DI<sup>3</sup>, for each part of gallium chloride that is reacted; hydrolyzing the pigment precursor chlorogallium phthalocyanine Type I by standard methods, for example acid pasting, whereby the pigment precursor is dissolved in concentrated sulfuric acid and then reprecipitated in a solvent, such as water, or a dilute ammonia solution, for example from about 10 to about 15 percent; and subsequently treating the resulting hydrolyzed pigment hydroxygallium phthalocyanine Type I with a solvent, such as N,N-dimethylformamide, present in an amount of from about 1 volume part to about 50 volume parts, and preferably about 15 volume parts for each weight part of pigment hydroxygallium phthalocyanine that is used by, for example, ball milling the Type I hydroxygallium phthalocyanine pigment in the presence of spherical glass beads, approximately 1 millimeter to 5 millimeters in diameter, at room temperature, about 25° C., for a period of from about 12 hours to about 1 week, and preferably about 24 hours.

The appropriate components, and processes of the above recited patents may be selected for the present disclosure in embodiments thereof.

## SUMMARY

Disclosed are imaging members with many of the advantages illustrated herein, such as extended lifetimes of service of, for example, in excess of about 3,500,000 imaging cycles; excellent electronic characteristics; stable electrical proper-

ties; low image ghosting; low background and/or minimal charge deficient spots (CDS); resistance to charge transport layer cracking upon exposure to the vapor of certain solvents; excellent surface characteristics; improved wear resistance; compatibility with a number of toner compositions; the avoidance of or minimal imaging member scratching characteristics; consistent  $V_r$  (residual potential) that is substantially flat or no change over a number of imaging cycles as illustrated by the generation of known PIDCs (Photo-Induced Discharge Curve); minimum cycle up in residual potential; acceptable background voltage that is, for example, a minimum background voltage of about 2.6 milliseconds after exposure of the photoconductor to a light source; rapid PIDCs together with low residual voltages, and the like.

Also disclosed are layered photoresponsive imaging members which are responsive to near infrared radiation of from about 700 to about 900 nanometers.

Further disclosed are layered flexible photoresponsive imaging members with sensitivity to visible light.

Moreover, disclosed are layered belt photoresponsive or photoconductive imaging members with mechanically robust and solvent resistant charge transport layers.

Additionally disclosed are flexible imaging members with optional hole blocking layers comprised of metal oxides, phenolic resins, and optional phenolic compounds, and which phenolic compounds contain at least two, and more specifically, two to ten phenol groups or phenolic resins with, for example, a weight average molecular weight ranging from about 500 to about 3,000 permitting, for example, a hole blocking layer with excellent efficient electron transport which usually results in a desirable photoconductor low residual potential  $V_{low}$ .

Also disclosed are layered flexible belt photoreceptors wherein there is permitted the prevention of  $V_r$  cycle up, caused primarily by photoconductor aging, for numerous imaging cycles, and layered flexible belt photoreceptors, and where the resulting imaging members exhibit low background and/or minimal CDS; and the prevention of  $V_r$  cycle up, caused primarily by photoconductor aging, for numerous imaging cycles.

## EMBODIMENTS

Aspects of the present disclosure relate to an imaging member comprising an optional supporting substrate, a photogenerating layer, and at least one charge transport layer, and wherein the photogenerating layer contains at least one thiophosphate, and an overcoating layer in contact with and contiguous to the charge transport layer, and which overcoating is comprised of an acrylated polyol, a polyalkylene glycol, a crosslinking component, and a charge transport component; an imaging member wherein the photogenerating layer is comprised of at least one photogenerating pigment and a dialkyldithiophosphate, and a crosslinked overcoating generated in the presence of a catalyst by the reaction of a polyol, a glycol, a crosslinking component, and a charge transport component to form a polymer network; a flexible photoconductive member comprised in sequence of a substrate, a photogenerating layer, and at least one charge transport layer comprised of at least one charge transport component, and wherein the photogenerating layer is comprised of at least one photogenerating pigment, and a thiophosphate

5

10

15

20

25

30

35

40

45

50

55

60

65



wherein  $R_1$ ,  $R_2$ ,  $R_3$ ,  $R_4$ ,  $R_5$  and  $R_6$  each independently represents at least one of a hydrogen atom, and a suitable hydrocarbon; and an overcoating in contact with and contiguous to the top or uppermost charge transport layer, and which overcoating is formed by the reaction of an acrylate polyol, a polyalkylene glycol, a crosslinking agent, and a charge transport compound in the presence of a catalyst resulting in a polymeric network primarily containing the acrylate polyol, the crosslinking agent, the glycol, and the charge transport compound; a photoconductor comprising a supporting substrate, a photogenerating layer, at least one charge transport layer, and wherein the photogenerating layer is comprised of at least one photogenerating pigment, and a dialkyldithiophosphate encompassed by



wherein  $R_1$ ,  $R_2$ ,  $R_3$ ,  $R_4$ ,  $R_5$  and  $R_6$  each independently represents a hydrogen atom, a suitable hydrocarbon, or mixtures thereof; and wherein the photogenerating layer and the charge transport layer include a resin binder; wherein at least one charge transport layer is from 2 to about 5, and the photogenerating layer is situated between the substrate and at least one charge transport; and a layer in contact with and contiguous to the top charge transport layer, and which layer is comprised of a crosslinked polymeric network; a member wherein the acrylated polyol is represented by



where  $R_s$  represents  $CH_2CR_1CO_2-$ ; where  $t=0$  to 1 and represents the mole fraction acrylic groups on available sites; where  $[R_s-CH_2]$ , can be located in linear or branched portions of  $R_a$ ,  $R_b$ ,  $R_c$ , and  $R_d$ ; where  $R_a$  and  $R_c$  independently represent at least one of a linear alkyl group, a linear alkoxy group, a branched alkyl group, and a branched alkoxy group, wherein each alkyl and alkoxy group contain, for example, from about 1 to about 20 carbon atoms;  $R_b$  and  $R_d$  independently represent at least one of an alkyl and alkoxy wherein the alkyl and the alkoxy each contain from about 1 to about 20 carbon atoms; and  $m$ ,  $n$ ,  $p$ , and  $q$  represent mole fractions of from 0 to 1, such that  $n+m+p+q=1$ ; a photoconductor wherein the overcoating acrylated polyol is represented by



where  $R_s$  represents  $CH_2CR_1CO_2-$ ; where  $t=0$  to 1 and represents the mole fraction acrylic groups on available sites; where  $[R_s-CH_2]$ , can be located in linear or branched portions of  $R_a$ ,  $R_b$ ,  $R_c$ , and  $R_d$ ; where  $R_a$  and  $R_c$  independently represent at least one of an alkyl group, an alkoxy group, a branched alkyl group, and a branched alkoxy group, wherein each alkyl and alkoxy group contain from about 1 to about 12 carbon atoms;  $R_b$  and  $R_d$  independently represent at least one of an alkyl and alkoxy wherein the alkyl and the alkoxy each contain from about 1 to about 12 carbon atoms; and  $m$ ,  $n$ ,  $p$ , and  $q$  represent mole fractions of from, for example, 0 to 1, such that  $n+m+p+q=1$ ; and wherein the overcoating primarily contains an acrylate polyol, a polyalkylene, a glycol, crosslinking agent, and a charge transport compound; an imaging member wherein at least one charge transport layer further contains a silanol; a flexible photoconductor comprised in sequence of a substrate, a photogenerating layer, and at least one charge transport layer comprised of at least one charge transport component, and wherein the at least one charge transport layer is comprised of hole transport molecules and at least one dialkyldithiophosphate, or wherein the dialkyldithiophosphate is present in the photogenerating layer



wherein  $R_1$ ,  $R_2$ ,  $R_3$ ,  $R_4$ ,  $R_5$  and  $R_6$  each independently represents at least one of a hydrogen atom, and a suitable hydrocarbon, such as alkyl, alkoxy, aryl, substituted derivatives thereof, and the like; and an overcoating layer in contact with and contiguous to the top charge transport layer, and which overcoating layer is formed by the reaction of an acrylate polyol, a polyalkylene, a crosslinking agent, and a charge

transport compound in the presence of a catalyst resulting in a polymeric network primarily containing the acrylate polyol, the glycol, the crosslinking component or agent, and charge transport compound; an imaging wherein the overcoating charge transport component is



wherein  $m$  is zero or 1;  $Z$  is selected from the group consisting of at least one of



wherein  $n$  is 0 or 1;  $Ar$  is selected from the group consisting of at least one of



$R$  is selected from the group consisting of at least one of  $-CH_3$ ,  $-C_2H_5$ ,  $-C_3H_7$ , and  $C_4H_9$ , and  $Ar'$  is selected from the group consisting of at least one of



and  $X$  is selected from the group consisting of at least one of





wherein S is zero, 1, or 2; a photoconductor comprising a substrate, a photogenerating layer, and at least one charge transport layer, for example wherein at least one is two, comprised of at least one charge transport component, and wherein the at least one charge transport layer, especially the first or second layer, is comprised of hole transport molecules and a thiophosphate represented by formulas/structures



wherein R<sub>1</sub>, R<sub>2</sub>, R<sub>3</sub>, R<sub>4</sub>, R<sub>5</sub> and R<sub>6</sub> each independently represents a hydrogen atom; alkyl, alkoxy, or aryl, and wherein at least one charge transport layer is comprised of from 2 to about 4 layers, and wherein 1 layer, 2 layers, 3 layers, or 4 charge transport layers contain a thiophosphate, or where the photogenerating layer contains the thiophosphate; and a layer in contact with and contiguous to the top charge transport layer, and which layer is formed by the reaction of an acrylate polyol, a polyalkylene glycol, a crosslinking agent, and a charge transport compound, and a catalyst resulting in a polymeric network where the amount of the thiophosphate in the photogenerating layer or CTL depends on a number of factors, generally however, this amount is from 0.1 to about 40, 5 to about 25, 5 to about 10, or 1 to about 15 weight percent. More specifically, at least one of R<sub>1</sub>, R<sub>2</sub>, R<sub>3</sub>, R<sub>4</sub>, R<sub>5</sub> and R<sub>6</sub> represents a hydrogen atom; an alkyl group with, for example, from 1 to about 20 carbon atoms; a cycloalkyl group with, for example, from 6 to about 26 carbon atoms; hydrocarbyl with, for example, from about 3 to about 20 carbon atoms containing an ester, an ether, an alcohol or a carboxyl group; a straight chain or branched alkyl with, for example, from 2 to about 18 carbon atoms; and the like.

In embodiments, for the thiophosphates, which can in embodiments be included in the photogenerating layer at least one of R<sub>1</sub>, R<sub>2</sub>, R<sub>3</sub>, R<sub>4</sub>, R<sub>5</sub> and R<sub>6</sub> represents a hydrogen atom; alkyl with, for example, from 1 to about 12 carbon atoms; cycloalkyl with, for example, from about 6 to about 20 carbon atoms; aryl, alkylaryl or arylalkyl groups with from

about 6 to about 50 carbon atoms; a hydrocarbyl group containing, for example, from about 5 to about 15 carbon atoms, and containing an ester, ether, alcohol or carboxyl group; and an alkyl group which may be straight, chain or branched with, for example, from about 2 to about 15 carbon atoms, or from about 3 to about 8 carbon atoms. Examples of alkyl and alkoxy groups include methyl, ethyl, propyl, isopropyl, butyl, isobutyl, pentyl, hexyl ethylhexyl, derivatives thereof, and the like, and mixtures thereof, and the corresponding alkoxydes. 5 Aryl examples are phenyl, naphthyl; aryl substituted with, for example, alkyl and alkoxy, and derivatives thereof. Examples of hydrocarbyl group containing, for example, from about 5 to about 15 carbon atoms, and containing an ester, ether, alcohol or carboxyl group.

Specific examples of metal dialkyldithiophosphates include molybdenum di(2-ethylhexyl)dithiophosphate, zinc diethyldithiophosphate, antimony diamyldithiophosphate, and the like. Commercial zinc dialkyldithiophosphates include ELCOTM 102, 103, 108, 114, 11, and 121, available from Elco Corporation, Cleveland, Ohio. A number of the thiophosphates contain a certain amount of petroleum distillates, mineral oils such as ValPar500TM, available from Valero Energy Corporation, San Antonio, Tex. Commercial molybdenum dialkyldithiophosphates include MOLYVAN LTM (molybdenum di(2-ethylhexyl)phosphorodithioate), available from R.T. Vanderbilt Company, Inc., Norwalk, Conn. Commercial antimony dialkyldithiophosphates include VANLUBE™ 622 and 648 (antimony dialkylphosphorodithioate), available from R.T. Vanderbilt Company, Inc., Norwalk, Conn.

30 Various effective amounts of the thiophosphates, which in embodiments function primarily as permitting excellent photoconductor electricals, although in theory there could be interactions between the thiophosphates and other components present, can be added to each charge transport layer and/or to the photogenerating layer components, such as from about 0.01 to about 30 weight percent, from about 0.1 to about 10 weight percent, or from about 0.5 to about 5 weight percent in the charge transport layer or layers; and from about 0.1 to about 40 weight percent, from about 1 to about 20 weight percent, or from about 5 to about 15 weight percent in the photogenerating layer.

Also disclosed are imaging members comprising an optional supporting substrate, a photogenerating layer containing a silanol, and at least one charge transport layer comprised of at least one charge transport component and an overcoating layer; a photoconductor comprising a supporting substrate, a photogenerating layer comprised of a photogenerating component and a silanol, and at least one charge transport layer comprised of at least one charge transport component, and wherein the silanol is selected from the group comprised of at least one of



11



12



and wherein R and R' are independently a suitable hydrocarbon like alkyl, alkoxy, aryl, and substituted derivatives thereof, and mixtures thereof, and a crosslinked overcoating in contact with and contiguous to the charge transport, and which overcoating is comprised of a charge transport compound, a polymer, and a crosslinking component; a photoconductor comprised in sequence of a supporting substrate, a photogenerating layer comprised of at least one photogenerating pigment, and a silanol; thereover a charge transport layer comprised of at least one charge transport component, and wherein the silanol is selected from the group comprised of at least one of the following; and a layer in contact with and contiguous to the top charge transport layer, and which layer is comprised of a crosslinked polymer which can be formed by the reaction of an acrylate polyol, a polyalkylene glycol, a crosslinking agent, and a charge transport compound in the presence of a catalyst resulting in a polymeric network primarily containing the acrylate polyol, the glycol, the crosslinking agent, and the charge transport compound wherein the silanol is

wherein R and R' are independently a suitable hydrocarbon, and wherein the silanol is present in an amount of from about 0.1 to about 40 weight percent; a photoconductor wherein the acrylated polyol is represented by



where  $R_s$  represents  $CH_2CR_1CO_2-$ ; where  $t=0$  to 1 and represents the mole fraction acrylic groups on available sites;

where  $[R_s-CH_2]_s$  can be located in linear or branched portions of  $R_a$ ,  $R_b$ ,  $R_c$ , and  $R_d$ ; where  $R_a$  and  $R_c$  independently represent at least one of a linear alkyl group, a linear alkoxy group, a branched alkyl group, and a branched alkoxy group wherein each alkyl and alkoxy group contain from about 1 to about 20 carbon atoms;  $R_b$  and  $R_d$  independently represent at least one of an alkyl and alkoxy wherein the alkyl and the alkoxy each contain from about 1 to about 20 carbon atoms; and  $m$ ,  $n$ ,  $p$ , and  $q$  represent mole fractions of from 0 to 1, such that  $n+m+p+q=1$ ; a photoconductor comprising an optional substrate, a photogenerating layer comprised of a photogenerating component and a silanol, and at least one charge transport layer comprised of at least one charge transport component, and wherein the photogenerating silanol is selected from the group comprised of the following formulas/structures



and wherein  $R$  and  $R'$  are independently alkyl, alkoxy, aryl, and substituted derivatives thereof, and mixtures thereof, and in contact with the charge transport layer a top overcoating layer of POC (protective overcoat); a photoconductor comprised in sequence of a supporting substrate, a photogenerat-

ing layer comprised of at least one photogenerating pigment, and a silanol, and thereover at least one charge transport layer comprised of at least one charge transport component, and wherein the silanol is selected from the group comprised of the following formulas/structures



wherein  $R$  and  $R'$  are independently a suitable hydrocarbon, and wherein the silanol is present in an amount of from about 0.1 to about 40 weight percent, and in contact with the charge transport layer a top overcoating layer or TOC, and which overcoating contains primarily an acrylated polyol, a polyalkylene glycol, wherein alkylene contains, for example, from 1 to about 10 carbon atoms, and more specifically, from 1 to about 4 carbon atoms, a charge transport, such as a hole transport compound, and minor amounts of a catalyst and a crosslinking agent; a flexible imaging member comprising a supporting substrate, a photogenerating layer, and at least two charge transport layers, at least one photogenerating or charge transport containing a silanol of the formulas, which silanols can also be referred to as polyhedral oligomeric silsesquioxane (POSS) silanols



wherein R and R' are independently selected from the group comprised of a suitable hydrocarbon, such as alkyl, alkoxy, aryl, and substituted derivatives thereof, and mixtures thereof with, for example, from 1 to about 36 carbon atoms like phenyl, methyl, vinyl, allyl, isobutyl, isoocetyl, cyclopentyl, cyclohexyl, cyclohexenyl-3-ethyl, epoxycyclohexyl-4-ethyl, fluorinated alkyl such as  $\text{CF}_3\text{CH}_2\text{CH}_2$ — and  $\text{CF}_3(\text{CF}_2)_5\text{CH}_2\text{CH}_2$ —, methacrylolpropyl, norbornenylethyl, and the like; and also wherein the R groups includes phenyl, isobutyl, isoocetyl, cyclopentyl, cyclohexyl and the like; desired R' group includes methyl, vinyl, fluorinated alkyl, and the like, and in contact with the charge transport layer a top overcoating crosslinked layer comprised of a mixture of polyols, such as a mixture of an acrylated polyol and an alkylene glycol, a charge transport compound, a crosslinking agent, and which overcoating layer is formed in the presence of an acid catalyst; a photoconductor comprised of a photogenerating layer, and at least one charge transport layer, and wherein the photogenerating layer contains at least one silanol as illustrated herein; or wherein both the photogenerating layer and the at least one charge transport layer contains at least one silanol as

- illustrated herein, or wherein the charge transport layers have an absence of a silanol, and such a silanol is included in the photogenerating layer and in contact with the charge transport layer a top protective crosslinked overcoating layer as illustrated herein; an imaging member comprising a supporting substrate, a photogenerating layer thereover, and at least one charge transport layer comprised of at least one charge transport component, at least one silanol of the formula illustrated herein wherein R and R' are independently alkyl, alkoxy, or aryl, or mixtures thereof like phenyl, methyl, vinyl, allyl, isobutyl, isoocetyl, cyclopentyl, cyclohexyl, cyclohexenyl-3-ethyl, epoxycyclohexyl-4-ethyl, fluorinated alkyl such as  $\text{CF}_3\text{CH}_2\text{CH}_2$ — and  $\text{CF}_3(\text{CF}_2)_5\text{CH}_2\text{CH}_2$ —, methacrylolpropyl, or norbornenylethyl; a photoconductive member comprised of a substrate, a photogenerating layer thereover, at least one to about three charge transport layers thereover, a hole blocking layer, an adhesive layer wherein in embodiments the adhesive layer is situated between the photogenerating layer and the hole blocking layer, and wherein at least one of the charge transport layers and the photogenerating layer contain a silanol, or wherein the silanol is contained solely in the photogenerating layer with the photogenerating layer including a photogenerating component, such as a photogenerating pigment and a resin binder, and the at least one charge transport layer including at least one charge transport component, such as a hole transport component, a resin binder, and known additives like antioxidants, and in contact with the entire surface of the charge transport layer a top overcoating protective layer as illustrated herein.
- The photoconductors illustrated herein can include in the photogenerating layer or the charge transport layer a dialkylidithiophosphate such as those represented by the following formulas/structures



wherein R<sub>1</sub>, R<sub>2</sub>, R<sub>3</sub>, R<sub>4</sub>, R<sub>5</sub> and R<sub>6</sub> each independently represents a hydrogen atom, a suitable hydrocarbon like alkyl, cycloalkyl, aryl, alkylaryl or arylalkyl, and mixtures thereof.

In embodiments thereof there is disclosed a photoconductive imaging member comprised of a supporting substrate, a photogenerating layer thereover, a charge transport layer, and an overcoating polymer layer; a photoconductive member with a photogenerating layer of a thickness of about 1 to about 10 microns, at least one transport layer each of a thickness of from about 5 to about 100 microns; a xerographic imaging apparatus containing a charging component, a development component, a transfer component, and a fixing component, and wherein the apparatus contains a photoconductive imaging member comprised of a supporting substrate,

and thereover a layer comprised of a photogenerating pigment and a charge transport layer or layers, and thereover an overcoating layer, and where the transport layer is of a thickness of from about 40 to about 75 microns; a member wherein the silanol or dialkyldithiophosphate is present in an amount of from about 0.1 to about 40 weight percent, or from about 6 to about 20 weight percent; a member wherein the photogenerating layer contains a photogenerating pigment present in an amount of from about 10 to about 95 weight percent; a member wherein the thickness of the photogenerating layer is from about 1 to about 4 microns; a member wherein the photogenerating layer contains an inactive polymer binder; a member wherein the binder is present in an amount of from about 50 to about 90 percent by weight, and wherein the total of all layer components is about 100 percent; a member wherein the photogenerating component is a hydroxygallium phthalocyanine that absorbs light of a wavelength of from about 370 to about 950 nanometers; an imaging member wherein the supporting substrate is comprised of a conductive substrate comprised of a metal; an imaging member wherein the conductive substrate is aluminum, aluminized polyethylene terephthalate or titanized polyethylene terephthalate; an imaging member wherein the photogenerating resinous binder is selected from the group consisting of known suitable polymers like polyesters, polyvinyl butyral, polycarbonates, polystyrene-b-polyvinyl pyridine, and polyvinyl formals; an imaging member wherein the photogenerating pigment is a metal free phthalocyanine; an imaging member wherein each of the charge transport layers, especially a first and second layer, or a single charge transport layer and the charge transport compound in the overcoating layer comprises



wherein X is selected from the group consisting of alkyl, alkoxy, and halogen, such as methyl and chloride; an imaging member wherein alkyl and alkoxy contain from about 1 to about 15 carbon atoms; an imaging member wherein alkyl contains from about 1 to about 5 carbon atoms; an imaging member wherein alkyl is methyl; an imaging member wherein each or at least one of the charge transport layers, especially a first and second charge transport layer, or a single charge transport layer, and the overcoating charge transport compound comprises



wherein X and Y are independently alkyl, alkoxy, aryl, a halogen, or mixtures thereof; an imaging member wherein, for example, alkyl and alkoxy contains from about 1 to about 15 carbon atoms; alkyl contains from about 1 to about 5 carbon atoms; and wherein the resinous binder is selected

from the group consisting of polycarbonates and polystyrene; an imaging member wherein the photogenerating pigment present in the photogenerating layer is comprised of chlorogallium phthalocyanine, or Type V hydroxygallium phthalocyanine prepared by hydrolyzing a gallium phthalocyanine precursor by dissolving the hydroxygallium phthalocyanine in a strong acid, and then reprecipitating the resulting dissolved precursor in a basic aqueous media; removing the ionic species formed by washing with water; concentrating the resulting aqueous slurry comprised of water and hydroxygallium phthalocyanine to a wet cake; removing water from the wet cake by drying; and subjecting the resulting dry pigment to mixing with the addition of a second solvent to cause the formation of the hydroxygallium phthalocyanine; an imaging member wherein the Type V hydroxygallium phthalocyanine has major peaks, as measured with an X-ray diffractometer, at Bragg angles (2 theta+/-0.2°) 7.4, 9.8, 12.4, 16.2, 17.6, 18.4, 21.9, 23.9, 25.0, 28.1 degrees, and the highest peak at 7.4 degrees; a method of imaging wherein the imaging member is exposed to light of a wavelength of from about 400 to about 950 nanometers; a member wherein the photogenerating layer is situated between the substrate and the charge transport; a member wherein the charge transport layer is situated between the substrate and the photogenerating layer, and wherein the number of charge transport layers is two; a member wherein the photogenerating layer is of a thickness of from about 5 to about 25 microns; a member wherein the photogenerating component amount is from about 0.05 weight percent to about 20 weight percent, and wherein the photogenerating pigment is dispersed in from about 10 weight percent to about 80 weight percent of a polymer binder; a member wherein the thickness of the photogenerating layer is from about 1 to about 11 microns; a member wherein the photogenerating and charge transport layer components are contained in a polymer binder; a member wherein the binder is present in an amount of from about 50 to about 90 percent by weight, and wherein the total of the layer components is about 100 percent; wherein the photogenerating resinous binder is selected from the group consisting of polyesters, polyvinyl butyral, polycarbonates, polystyrene-b-polyvinyl pyridine, and polyvinyl formals; an imaging member wherein the photogenerating component is Type V hydroxygallium phthalocyanine, or chlorogallium phthalocyanine, and the charge transport layer and/or overcoating contains a hole transport of N,N'-diphenyl-N,N'-bis(3-methylphenyl)-1,1'-biphenyl-4,4'-diamine, N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis-(4-isopropylphenyl)-[p-terphenyl]-4,4"-diamine, N,N'-bis(4-butylphenyl)-N,N'-bis-(2-ethyl-6-methylphenyl)-[p-terphenyl]-4,4"-diamine, N,N'-bis(4-butylphenyl)-N,N'-bis-(2,5-dimethylphenyl)-[p-terphenyl]-4,4"-diamine, N,N'-diphenyl-N,N'-bis(3-chlorophenyl)-[p-terphenyl]-4,4"-diamine molecules, and wherein the hole transport resinous binder is selected from the group consisting of polycarbonates and polystyrene; an imaging member wherein the photogenerating layer contains a metal free phthalocyanine; an imaging member wherein the photogenerating layer contains an alkoxygallium phthalocyanine; a photoconductive imaging member with a blocking layer contained as a coating on a substrate, and an adhesive layer coated on the blocking layer; an imaging member further containing an adhesive layer and a hole blocking layer; a color method of imaging which comprises generating an electrostatic latent image on the imaging member, developing the latent image, transferring, and fixing the developed electrostatic image to a suitable substrate; photoconductive imaging members comprised of a supporting substrate, a photogenerating layer, a hole transport

19

layer, and a top overcoating layer in contact with the hole transport layer, or in embodiments in contact with the photo-generating layer, and in embodiments wherein a plurality of charge transport layers are selected, such as, for example, from 2 to about 10, and more specifically 2 may be selected; and a photoconductive imaging member comprised of an optional supporting substrate, a photogenerating layer, and a first, second, and third charge transport layer.

Examples of POSS silanols wherein "throughout POSS" refers to polyhedral oligomeric silsesquioxane silanols include isobutyl-POSS cyclohexenyldimethylsilyldisilanol or isobutyl-polyhedral oligomeric silsesquioxane cyclohexenyldimethylsilyldisilanol ( $C_{38}H_{84}O_{12}Si_8$ ), cyclopentyl-POSS dimethylphenyldisilanol ( $C_{43}H_{76}O_{12}Si_8$ ), cyclohexyl-POSS dimethylvinyldisilanol ( $C_{46}H_{88}O_{12}Si_8$ ), cyclopentyl-POSS dimethylvinyldisilanol ( $C_{39}H_{74}O_{12}Si_8$ ), isobutyl-POSS dimethylvinyldisilanol ( $C_{32}H_{74}O_{12}Si_8$ ), cyclopentyl-POSS disilanol ( $C_{40}H_{74}O_{13}Si_8$ ), isobutyl-POSS disilanol ( $C_{32}H_{74}O_{13}Si_8$ ), isobutyl-POSS epoxycyclohexyldisilanol ( $C_{38}H_{84}O_{13}Si_8$ ), cyclopentyl-POSS fluoro(3)disilanol ( $C_{40}H_{75}F_3O_{12}Si_8$ ), cyclopentyl-POSS fluoro(13)disilanol ( $C_{45}H_{75}F_{13}O_{12}Si_8$ ), isobutyl-POSS fluoro(13)disilanol ( $C_{38}H_{75}F_{13}O_{12}Si_8$ ), cyclohexyl-POSS methacryldisilanol ( $C_{51}H_{96}O_{14}Si_8$ ), cyclopentyl-POSS methacryldisilanol ( $C_{44}H_{82}O_{14}Si_8$ ), isobutyl-POSS methacryldisilanol ( $C_{37}H_{82}O_{14}Si_8$ ), cyclohexyl-POSS monosilanol ( $C_{42}H_{78}O_{13}Si_8$ ), cyclopentyl-POSS monosilanol (Schwabinol,  $C_{35}H_{64}O_{13}Si_8$ ), isobutyl-POSS monosilanol ( $C_{28}H_{64}O_{13}Si_8$ ), cyclohexyl-POSS norbornenylethyldisilanol ( $C_{53}H_{98}O_{12}Si_8$ ), cyclopentyl-POSS norbornenylethyldisilanol ( $C_{46}H_{84}O_{12}Si_8$ ), isobutyl-POSS norbornenylethyldisilanol ( $C_{39}H_{84}O_{12}Si_8$ ), cyclohexyl-POSS TMS disilanol ( $C_{45}H_{88}O_{12}Si_8$ ), isobutyl-POSS TMS disilanol ( $C_{31}H_{74}O_{12}Si_8$ ), cyclohexyl-POSS trisilanol ( $C_{42}H_{80}O_{12}Si_7$ ), cyclopentyl-POSS trisilanol ( $C_{35}H_{66}O_{12}Si_7$ ), isobutyl-POSS trisilanol ( $C_{28}H_{66}O_{12}Si_7$ ), isoctyl-POSS trisilanol ( $C_{56}H_{122}O_{12}Si_7$ ), phenyl-POSS trisilanol ( $C_{42}H_{38}O_{12}Si_7$ ), and the like, all commercially available from Hybrid Plastics, Fountain Valley, Calif. In embodiments, the POSS silanol is a phenyl-POSS trisilanol, or phenyl-polyhedral oligomeric silsesquioxane trisilanol of the following formula/structure



The POSS silanol can contain from about 7 to about 20 silicon atoms, or from about 7 to about 12 silicon atoms. The  $M_w$  of

20

the POSS silanol is, for example, from about 700 to about 2,000, or from about 800 to about 1,300.

Disclosed as silanol examples are



where R is phenyl;





In embodiments, silanols that can be selected are free of POSS. Examples of such silanols include dimethyl(thien-2-yl)silanol, tris(isopropoxy)silanol, tris(tert-butoxy)silanol, tris(tert-pentoxy)silanol, tris(o-tolyl)silanol, tris(1-naphthyl)silanol, tris(2,4,6-trimethylphenyl)silanol, tris(2-methoxyphenyl)silanol, tris(4-(dimethylamino)phenyl)silanol, tris(4-biphenyl)silanol, tris(trimethylsilyl)silanol, dicyclohexyltetrasilanol ( $C_{12}H_{26}O_5Si_2$ ), mixtures thereof, and the like.

The silanols selected for the members, devices, and photoconductors illustrated herein are stable primarily in view of the Si—OH substituents in that these substituents eliminate water to form siloxanes, that is Si—O—Si linkages. While not being limited by theory, it is believed that the silanol hindered structures at the other three bonds attached to the silicon render them stable for extended time periods, such as from at least one week to over two years. The silanols can be included in the charge transport layer solution or dispersion, or the photogenerating layer solution or dispersion that is, for example, dissolved therein, or alternatively the silanols can be added to the charge transport and/or the photogenerating layer.

Various suitable amounts of the silanols can be selected, such as from about 0.01 to about 50 percent by weight of solids throughout, or from about 1 to about 30 percent by weight, or from about 5 to about 20 percent by weight. The silanols can be dissolved in the charge transport layer solution and the photogenerating solution, or alternatively the silanol can simply be added to the formed charge transport layer and/or the formed photogenerating layer. In embodiments, the silanol is included in the known dispersion milling process when preparing the photogenerating layer.

For the photogenerating layer, although not desiring to be limited by theory, it is believed that the photogenerating pigment is modified with a hydrophobic moiety by the in situ attachment of a hydrophobic silanol onto the photogenerating pigment surface with the remainder of the silanol interacting with the resin binder thereby enabling the pigment to be readily dispersible during the dispersion milling process.

The thickness of the photoconductor substrate layer depends on many factors, including economical considerations, electrical characteristics, and the like, thus this layer may be of substantial thickness, for example over 3,000 microns, such as from about 1,000 to about 2,000 microns, from about 500 to about 900 microns, from about 300 to about 700 microns, or of a minimum thickness. In embodiments, the thickness of this layer is from about 75 microns to about 300 microns, or from about 100 microns to about 150 microns.

The substrate may be opaque or substantially transparent, and may comprise any suitable material. Accordingly, the substrate may comprise a layer of an electrically nonconductive or conductive material, such as an inorganic or an organic composition. As electrically nonconducting materials, there may be employed various resins known for this purpose including polyesters, polycarbonates, polyamides, polyurethanes, and the like, which are flexible as thin webs. An electrically conducting substrate may be any suitable metal of, for example, aluminum, nickel, steel, copper, and the like, or a polymeric material, as described above, filled with an electrically conducting substance, such as carbon, metallic powder, and the like, or an organic electrically conducting material. The electrically insulating or conductive substrate may be in the form of an endless flexible belt, a web, a rigid cylinder, a sheet, and the like. The thickness of the substrate layer depends on numerous factors, including strength desired and economical considerations. For a drum, as disclosed in a copending application referenced herein, this layer may be of substantial thickness of, for example, up to many centimeters or of a minimum thickness of less than a millimeter. Similarly, a flexible belt may be of substantial thickness of, for example, about 250 micrometers, or of minimum thickness of less than about 50 micrometers, provided there are no adverse effects on the final electrophotographic device.

In embodiments where the substrate layer is not conductive, the surface thereof may be rendered electrically conductive by an electrically conductive coating. The conductive coating may vary in thickness over substantially wide ranges depending upon the optical transparency, degree of flexibility desired, and economic factors.

Illustrative examples of substrates are as illustrated herein, and more specifically, layers selected for the imaging members of the present disclosure, and which substrates can be opaque or substantially transparent comprise a layer of insulating material including inorganic or organic polymeric materials, such as MYLAR® a commercially available polymer, MYLAR® containing titanium, a layer of an organic or inorganic material having a semiconductive surface layer, such as indium tin oxide or aluminum arranged thereon, or a conductive material inclusive of aluminum, chromium, nickel, brass, or the like. The substrate may be flexible, seamless, or rigid, and may have a number of many different configurations, such as for example, a plate, a cylindrical drum, a scroll, an endless flexible belt, and the like. In embodiments, the substrate is in the form of a seamless flexible belt. In some situations, it may be desirable to coat on the back of the substrate, particularly when the substrate is a flexible organic polymeric material, an anticurl layer, such as for example, polycarbonate materials commercially available as MAKROLON®.

The photogenerating layer in embodiments is comprised of a number of known photogenerating pigments, such as for example, about 50 weight percent of Type V hydroxygallium phthalocyanine or chlorogallium phthalocyanine, and about 50 weight percent of a resin binder like poly(vinyl chloride-co-vinyl acetate) copolymer, such as VMCH (available from Dow Chemical). Generally, the photogenerating layer can contain known photogenerating pigments, such as metal phthalocyanines, metal free phthalocyanines, alkylhydroxyl gallium phthalocyanines, hydroxygallium phthalocyanines, chlorogallium phthalocyanines, perylenes, especially bis (benzimidazo)perylene, titanyl phthalocyanines, and the like, and more specifically, vanadyl phthalocyanines, Type V hydroxygallium phthalocyanines, and inorganic components, such as selenium, selenium alloys, and trigonal selenium. The photogenerating pigment can be dispersed in a resin binder similar to the resin binders selected for the charge transport layer, or alternatively no resin binder need be present. Generally, the thickness of the photogenerating layer depends on a number of factors, including the thicknesses of the other layers, and the amount of photogenerating material contained in the photogenerating layer. Accordingly, this layer can be of a thickness of, for example, from about 0.05 micron to about 10 microns, and more specifically, from about 0.25 micron to about 2 microns when, for example, the photogenerating compositions are present in an amount of from about 30 to about 75 percent by volume. The maximum thickness of this layer in embodiments is dependent primarily upon factors, such as photosensitivity, electrical properties and mechanical considerations. The photogenerating layer binder resin is present in various suitable amounts, for example from about 1 to about 50 weight percent, and more specifically, from about 1 to about 10 weight percent, and which resin may be selected from a number of known polymers, such as poly(vinyl butyral), poly(vinyl carbazole), polyesters, polycarbonates, poly(vinyl chloride), polyacrylates and methacrylates, copolymers of vinyl chloride and vinyl acetate, phenolic resins, polyurethanes, poly(vinyl alcohol), polyacrylonitrile, polystyrene, and the like. It is desirable to select a coating solvent that does not substantially disturb or adversely affect the other previously coated layers of the device. Examples of coating solvents for the photogenerating layer are ketones, alcohols, aromatic hydrocarbons, halogenated aliphatic hydrocarbons, silanols, amines, amides, esters, and the like. Specific solvent examples are cyclohexanone, acetone, methyl ethyl ketone, methanol, ethanol, butanol, amyl alcohol, toluene, xylene, chlorobenzene, carbon tetrachloride, chloroform, methylene chloride, trichloroethylene, tetrahydrofuran, dioxane, diethyl ether, dimethyl formamide, dimethyl acetamide, butyl acetate, ethyl acetate, methoxyethyl acetate, and the like.

The photogenerating layer may comprise amorphous films of selenium and alloys of selenium and arsenic, tellurium, germanium, and the like; hydrogenated amorphous silicon; and compounds of silicon and germanium, carbon, oxygen, nitrogen, and the like fabricated by vacuum evaporation or deposition. The photogenerating layers may also comprise inorganic pigments of crystalline selenium and its alloys; Groups II to VI compounds; and organic pigments, such as quinacridones, polycyclic pigments, such as dibromoanthanthrone pigments, perylene and perinone diamines, polynuclear aromatic quinones, azo pigments including bis-, tri- and tetrakis-azos; and the like dispersed in a film forming polymeric binder, and fabricated by solvent coating techniques.

Infrared sensitivity can be desired for photoreceptors exposed to low cost semiconductor laser diode light exposure

devices where, for example, the absorption spectrum and photosensitivity of the phthalocyanines selected depend on the central metal atom thereof. Examples include oxyvanadium phthalocyanine, chloroaluminum phthalocyanine, copper phthalocyanine, oxytitanium phthalocyanine, chlorogallium phthalocyanine, hydroxygallium phthalocyanine, magnesium phthalocyanine, and metal free phthalocyanine. The phthalocyanines exist in many crystal forms, and have a strong influence on photogeneration.

In embodiments, examples of polymeric binder materials that can be selected as the matrix for the photogenerating layer are illustrated in U.S. Pat. No. 3,121,006, the disclosure of which is totally incorporated herein by reference. Examples of binders are thermoplastic and thermosetting resins, such as polycarbonates, polyesters, polyamides, polyurethanes, polystyrenes, polyarylsilanols, polyarylsulfones, polybutadienes, polysulfones, polysilanolsulfones, polyethylenes, polypropylenes, polyimides, polymethylpentenes, poly(phenylene sulfides), poly(vinyl acetate), polysiloxanes, polyacrylates, polyvinyl acetals, polyamides, polyimides, amino resins, phenylene oxide resins, terephthalic acid resins, phenoxy resins, epoxy resins, phenolic resins, polystyrene and acrylonitrile copolymers, poly(vinyl chloride), vinyl chloride and vinyl acetate copolymers, acrylate copolymers, alkyl resins, cellulosic film formers, poly(amideimide), styrene butadiene copolymers, vinylidene chloride-vinyl chloride copolymers, vinyl acetate-vinylidene chloride copolymers, styrene-alkyd resins, poly(vinyl carbazole), and the like. These polymers may be block, random or alternating copolymers.

The photogenerating composition or pigment is present in the resinous binder composition in various amounts. Generally, however, from about 5 percent by weight to about 90 percent by weight of the photogenerating pigment is dispersed in about 10 percent by weight to about 95 percent by weight of the resinous binder, or from about 20 percent by weight to about 50 percent by weight of the photogenerating pigment is dispersed in about 80 percent by weight to about 50 percent by weight of the resinous binder composition. In one embodiment, about 50 percent by weight of the photogenerating pigment is dispersed in about 50 percent by weight of the resinous binder composition.

Various suitable and conventional known processes may be used to mix, and thereafter apply the photogenerating layer coating mixture like spraying, dip coating, roll coating, wire wound rod coating, vacuum sublimation, and the like. For some applications, the photogenerating layer may be fabricated in a dot or line pattern. Removal of the solvent of a solvent-coated layer may be effected by any known conventional techniques such as oven drying, infrared radiation drying, air drying, and the like.

The coating of the photogenerating layer in embodiments of the present disclosure can be accomplished with spray, dip or wire-bar methods such that the final dry thickness of the photogenerating layer is as illustrated herein, and can be, for example, from about 0.01 to about 30 microns after being dried at, for example, about 40° C. to about 150° C. for about 15 to about 90 minutes. More specifically, a photogenerating layer of a thickness, for example, of from about 0.1 to about 30 microns, or from about 0.5 to about 2 microns can be applied to or deposited on the substrate, on other surfaces in between the substrate and the charge transport layer, and the like. A charge blocking layer or hole blocking layer may optionally be applied to the electrically conductive surface prior to the application of a photogenerating layer. When desired, an adhesive layer may be included between the charge blocking or hole blocking layer or interfacial layer,

and the photogenerating layer. Usually, the photogenerating layer is applied onto the blocking layer and a charge transport layer or plurality of charge transport layers are formed on the photogenerating layer. This structure may have the photogenerating layer on top of or below the charge transport layer.

In embodiments, a suitable known adhesive layer can be included in the photoconductor. Typical adhesive layer materials include, for example, polyesters, polyurethanes, and the like. The adhesive layer thickness can vary and in embodiments is, for example, from about 0.05 micrometer (500 Angstroms) to about 0.3 micrometer (3,000 Angstroms). The adhesive layer can be deposited on the hole blocking layer by spraying, dip coating, roll coating, wire wound rod coating, gravure coating, Bird applicator coating, and the like. Drying of the deposited coating may be effected by, for example, oven drying, infrared radiation drying, air drying, and the like.

As optional adhesive layers usually in contact with or situated between the hole blocking layer and the photogenerating layer, there can be selected various known substances inclusive of copolymers, polyamides, poly(vinyl butyral), poly(vinyl alcohol), polyurethane, and polyacrylonitrile. This layer is, for example, of a thickness of from about 0.001 micron to about 1 micron, or from about 0.1 micron to about 0.5 micron. Optionally, this layer may contain effective suitable amounts, for example from about 1 to about 10 weight percent, of conductive and nonconductive particles, such as zinc oxide, titanium dioxide, silicon nitride, carbon black, and the like, to provide, for example, in embodiments of the present disclosure further desirable electrical and optical properties.

The optional hole blocking or undercoat layers for the imaging members of the present disclosure can contain a number of components including known hole blocking components, such as amino silanes, doped metal oxides, TiSi, a metal oxide like titanium, chromium, zinc, tin and the like; a mixture of phenolic compounds and a phenolic resin, or a mixture of two phenolic resins, and optionally a dopant such as SiO<sub>2</sub>. The phenolic compounds usually contain at least two phenol groups, such as bisphenol A (4,4'-isopropylidenediphenol), E (4,4'-ethylidenebisphenol), F (bis(4-hydroxyphenyl)methane), M (4,4'-(1,3-phenylenediisopropylidene)bisphenol), P (4,4'-(1,4-phenylene diisopropylidene)bisphenol), S (4,4'-sulfonyldiphenol), and Z (4,4'-cyclohexylidenebisphenol); hexafluorobisphenol A (4,4'-hexafluoro isopropylidene) diphenol), resorcinol, hydroxyquinone, catechin, and the like.

The hole blocking layer can be, for example, comprised of from about 20 weight percent to about 80 weight percent, and more specifically, from about 55 weight percent to about 65 weight percent of a suitable component like a metal oxide, such as TiO<sub>2</sub>; from about 20 weight percent to about 70 weight percent, and more specifically, from about 25 weight percent to about 50 weight percent of a phenolic resin; from about 2 weight percent to about 20 weight percent, and more specifically, from about 5 weight percent to about 15 weight percent of a phenolic compound preferably containing at least two phenolic groups, such as bisphenol S; and from about 2 weight percent to about 15 weight percent, and more specifically, from about 4 weight percent to about 10 weight percent of a plywood suppression dopant, such as SiO<sub>2</sub>. The hole blocking layer coating dispersion can, for example, be prepared as follows. The metal oxide/phenolic resin dispersion is first prepared by ball milling or dynomilling until the median particle size of the metal oxide in the dispersion is less than about 10 nanometers, for example from about 5 to about 9 nanometers. To the above dispersion are added a phenolic

compound and dopant followed by mixing. The hole blocking layer coating dispersion can be applied by dip coating or web coating, and the layer can be thermally cured after coating. The hole blocking layer resulting is, for example, of a thickness of from about 0.01 micron to about 30 microns, and more specifically, from about 0.1 micron to about 8 microns. Examples of phenolic resins include formaldehyde polymers with phenol, p-tert-butylphenol, cresol, such as VARCUM® 29159 and 29101 (available from OxyChem Company), and DURITE® 97 (available from Borden Chemical); formaldehyde polymers with ammonia, cresol and phenol, such as VARCUM® 29112 (available from OxyChem Company); formaldehyde polymers with 4,4'-(1-methylethylidene)bisphenol, such as VARCUM® 29108 and 29116 (available from OxyChem Company); formaldehyde polymers with cresol and phenol, such as VARCUM® 29457 (available from OxyChem Company), DURITE® SD-423A, SD-422A (available from Borden Chemical); or formaldehyde polymers with phenol and p-tert-butylphenol, such as DURITE® ESD 556C (available from Borden Chemical).

The optional hole blocking layer may be applied to the substrate. Any suitable and conventional blocking layer capable of forming an electronic barrier to holes between the adjacent photoconductive layer (or electrophotographic imaging layer) and the underlying conductive surface of substrate may be selected.

The charge transport layer, which layer is generally of a thickness of from about 5 microns to about 75 microns, and more specifically, of a thickness of from about 10 microns to about 40 microns, components, and molecules include a number of known materials, such as aryl amines, of the following formula



45

wherein X is alkyl, alkoxy, aryl, a halogen, or mixtures thereof, or wherein each X is present on each of the four terminating rings; and especially those substituents selected from the group consisting of C<sub>1</sub> and CH<sub>3</sub>; and molecules of the following formula



wherein at least one of X, Y and Z are independently alkyl, alkoxy, aryl, a halogen, or mixtures thereof, and wherein either Y, Z, or both Y and Z can be present; N,N'-diphenyl-N,N'-bis(3-hydroxyphenyl)-[1,1'-biphenyl]-4,4'-diamine represented by



terphenyl arylamines as represented by



where each  $R_1$  and  $R_2$  is independently selected from the group consisting of at least one of —H, —OH,  $—C_nH_{2n+1}$  where  $n$  is from 1 to about 12, aralkyl, and aryl groups, the aralkyl and aryl groups having, for example, from about 6 to about 36 carbon atoms. The dihydroxy arylamine compounds can be free of any direct conjugation between the —OH groups and the nearest nitrogen atom through one or more aromatic rings. The expression “direct conjugation” refers, for example, to the presence of a segment, having the formula  $—(C=C)_n—C=C—$  in one or more aromatic rings directly between an —OH group and the nearest nitrogen atom. Examples of direct conjugation between the —OH groups and the nearest nitrogen atom through one or more aromatic rings include a compound containing a phenylene group having an —OH group in the ortho or para position (or 2 or 4 position) on the phenylene group relative to a nitrogen atom attached to the phenylene group or a compound containing a polyphenylene group having an —OH group in the ortho or para position on the terminal phenylene group relative to a nitrogen atom attached to an associated phenylene group. Examples of aralkyl groups include, for example,  $—C_nH_{2n-1}$ -phenyl groups where  $n$  is from about 1 to about 5, or from about 1 to about 10; examples of aryl groups include, for example, phenyl, naphthyl, biphenyl, and the like. In embodiments when  $R_1$  is —OH and each  $R_2$  is n-butyl, the resultant compound is  $N,N'$ -bis[4-n-butylphenyl]- $N,N'$ -di[3-hydroxyphenyl]-terphenyl-diamine. Also, in embodiments, the hole transport is soluble in the solvent selected for the formation of the overcoat layer.

Alkyl and alkoxy contain, for example, from 1 to about 25 carbon atoms, and more specifically, from 1 to about 12 carbon atoms, such as methyl, ethyl, propyl, butyl, pentyl, and the corresponding alkoxides. Aryl can contain from 6 to about 36 carbon atoms, such as phenyl, and the like. Halogen includes chloride, bromide, iodide and fluoride. Substituted alkyls, alkoxy, and aryls can also be selected in embodiments.

Examples of specific aryl amines include  $N,N'$ -diphenyl- $N,N'$ -bis(alkylphenyl)-1,1'-biphenyl-4,4'-diamine wherein alkyl is selected from the group consisting of methyl, ethyl, propyl, butyl, hexyl, and the like;  $N,N'$ -diphenyl- $N,N'$ -bis(halophenyl)-1,1'-biphenyl-4,4'-diamine wherein the halo

substituent is a chloro substituent;  $N,N'$ -bis(4-butylphenyl)- $N,N'$ -di-p-tolyl-[p-terphenyl]-4,4"-diamine,  $N,N'$ -bis(4-butylphenyl)-N,N'-di-m-tolyl-[p-terphenyl]-4,4"-diamine,  $N,N'$ -bis(4-butylphenyl)-N,N'-di-o-tolyl-[p-terphenyl]-4,4"-diamine,  $N,N'$ -bis(4-butylphenyl)-N,N'-bis-(4-isopropylphenyl)-[p-terphenyl]-4,4"-diamine,  $N,N'$ -bis(4-butylphenyl)-N,N'-bis-(2-ethyl-6-methylphenyl)-[p-terphenyl]-4,4"-diamine,  $N,N'$ -bis(4-butylphenyl)-N,N'-bis-(2,5-dimethylphenyl)-[p-terphenyl]-4,4"-diamine,  $N,N'$ -diphenyl- $N,N'$ -bis(3-chlorophenyl)-[p-terphenyl]-4,4"-diamine, and the like. Other known charge transport layer molecules can be selected, reference for example, U.S. Pat. Nos. 4,921,773 and 4,464,450, the disclosures of which are totally incorporated herein by reference.

15 The charge transport layer component can be selected as the charge transport compound for the photoconductor top overcoating layer.

Examples of the binder materials selected for the charge transport layers include components, such as those described

20 in U.S. Pat. No. 3,121,006, the disclosure of which is totally incorporated herein by reference. Specific examples of polymer binder materials include polycarbonates, polyarylates, acrylate polymers, vinyl polymers, cellulose polymers, polyesters, polysiloxanes, polyamides, polyurethanes, poly(cycloolefins), epoxies, and random or alternating copolymers thereof; and more specifically, polycarbonates such as poly(4,4'-isopropylidene-diphenylene)carbonate (also referred to as bisphenol-A-polycarbonate), poly(4,4'-cyclohexylidene-diphenylene)carbonate (also referred to as bisphenol-Z-polycarbonate), poly(4,4'-isopropylidene-3,3'-dimethyl-diphenyl)carbonate (also referred to as bisphenol-C-polycarbonate), and the like. In embodiments, electrically inactive binders are comprised of polycarbonate resins with a molecular weight of from about 20,000 to about 100,000, or 25 with a molecular weight  $M_w$  of from about 50,000 to about 100,000 preferred. Generally, the transport layer contains from about 10 to about 75 percent by weight of the charge transport material, and more specifically, from about 35 percent to about 50 percent of this material.

30 40 The charge transport layer or layers, and more specifically, a first charge transport in contact with the photogenerating layer, and thereover a top or second charge transport layer may comprise charge transporting small molecules dissolved or molecularly dispersed in a film forming electrically inert polymer such as a polycarbonate. In embodiments, “dissolved” refers, for example, to forming a solution in which the small molecule and silanol are dissolved in the polymer to form a homogeneous phase; and “molecularly dispersed in 35 embodiments” refers, for example, to charge transporting molecules dispersed in the polymer, the small molecules being dispersed in the polymer on a molecular scale. Various charge transporting or electrically active small molecules may be selected for the charge transport layer or layers. In 45 embodiments, charge transport refers, for example, to charge 50 transporting molecules as a monomer that allows the free charge generated in the photogenerating layer to be transported across the transport layer.

55 Examples of charge transporting molecules present in the charge transport layer in an amount of, for example, from 60 about 20 to about 55 weight percent, include, for example, pyrazolines such as 1-phenyl-3-(4'-diethylamino styryl)-5-(4"-diethylamino phenyl)pyrazoline; aryl amines such as  $N,N'$ -diphenyl- $N,N'$ -bis(3-methylphenyl)-(1,1'-biphenyl)-4,4'-diamine,  $N,N'$ -bis(4-butylphenyl)- $N,N'$ -di-p-tolyl-[p-terphenyl]-4,4"-diamine,  $N,N'$ -bis(4-butylphenyl)- $N,N'$ -di-m-tolyl-[p-terphenyl]-4,4"-diamine,  $N,N'$ -bis(4-butylphenyl)- $N,N'$ -di-o-tolyl-[p-terphenyl]-4,4"-diamine,  $N,N'$ -bis(4-

butylphenyl)-N,N'-bis-(4-isopropylphenyl)-[p-terphenyl]-4,4"-diamine, N,N'-bis(4-butylphenyl)-N,N'-bis-(2-ethyl-6-methylphenyl)-[p-terphenyl]-4,4"-diamine, N,N'-bis(4-butylphenyl)-N,N'-bis-(2,5-dimethylphenyl)-[p-terphenyl]-4,4"-diamine, N,N'-diphenyl-N,N'-bis(3-chlorophenyl)-[p-terphenyl]-4,4"-diamine; hydrazones such as N-phenyl-N-methyl-3-(9-ethyl)carbazyl hydrazone, and 4-diethyl amino benzaldehyde-1,2-diphenyl hydrazone; and oxadiazoles, such as 2,5-bis(4-N,N'-diethylaminophenyl)-1,2,4-oxadiazole, stilbenes, and the like. However, in embodiments to minimize or avoid cycle-up in equipment, such as printers, with high throughput, the charge transport layer should be substantially free (less than about two percent) of di or triaminotriphenyl methane. A small molecule charge transporting compound that permits injection of holes into the photogenerating layer with high efficiency, and transports them across the charge transport layer with short transit times, and which layer contains a binder and a silanol includes N,N'-diphenyl-N,N'-bis(3-methylphenyl)-(1,1'-biphenyl)-4,4"-diamine, N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis(4-isopropylphenyl)-[p-terphenyl]-4,4"-diamine, N,N'-bis(4-butylphenyl)-N,N'-bis-(2-ethyl-6-methylphenyl)-[p-terphenyl]-4,4"-diamine, N,N'-bis(4-butylphenyl)-N,N'-bis-(2,5-dimethylphenyl)-[p-terphenyl]-4,4"-diamine, and N,N'-diphenyl-N,N'-bis(3-chlorophenyl)-[p-terphenyl]-4,4"-diamine, or mixtures thereof. If desired, the charge transport material in the charge transport layer may comprise a polymeric charge transport material, or a combination of a small molecule charge transport material and a polymeric charge transport material.

A number of processes may be used to mix, and thereafter apply the charge transport layer or layers coating mixture to the photogenerating layer. Typical application techniques include spraying, dip coating, roll coating, wire wound rod coating, and the like. Drying of the charge transport deposited coating may be effected by any suitable conventional technique such as oven drying, infrared radiation drying, air drying, and the like.

The thickness of each of the charge transport layers in embodiments is from about 5 to about 75 microns, but thicknesses outside this range may, in embodiments, also be selected. The charge transport layer should be an insulator to the extent that an electrostatic charge placed on the hole transport layer is not conducted in the absence of illumination at a rate sufficient to prevent formation and retention of an electrostatic latent image thereon. In general, the ratio of the thickness of the charge transport layer to the photogenerating layer can be from about 2:1 to 200:1, and in some instances 400:1. The charge transport layer is substantially nonabsorbing to visible light or radiation in the region of intended use, but is electrically "active" in that it allows the injection of photogenerated holes from the photoconductive layer, or photogenerating layer, and allows these holes to be transported through itself to selectively discharge a surface charge on the surface of the active layer.

The thickness of the continuous charge transport overcoat layer selected depends upon the abrasiveness of the charging (bias charging roll), cleaning (blade or web), development (brush), transfer (bias transfer roll), and the like in the system employed, and this thickness can be up to about 10 micrometers. In embodiments, this thickness for each layer is from about 1 micrometer to about 5 micrometers. Various suitable and conventional methods may be used to mix, and thereafter apply the overcoat layer coating mixture to the charge trans-

port layer. Typical application techniques include spraying, dip coating, roll coating, wire wound rod coating, and the like. Drying of the deposited coating may be effected by any suitable conventional technique, such as oven drying, infrared radiation drying, air drying, and the like. The dried overcoating layer of this disclosure should transport holes during imaging and should not have too high a free carrier concentration.

The top charge transport layer can comprise the same components as the charge transport layer wherein the weight ratio between the charge transporting small molecules, and the suitable electrically inactive resin binder is less, such as for example, from about 0/100 to about 60/40, or from about 20/80 to about 40/60.

The photoconductors disclosed herein include a protective overcoating layer (POC) usually in contact with and contiguous to the charge transport layer. This POC layer is comprised of components that include (i) an acrylated polyol, and (ii) an alkylene glycol polymer, such as polypropylene glycol where the proportion of the acrylated polyol to the polypropylene glycol is, for example, from about 0.1:0.9 to about 0.9:0.1, at least one transport compound, and at least one crosslinking agent. The overcoat composition can comprise as a first polymer an acrylated polyol with a hydroxyl number of from about 10 to about 20,000; a second polymer of an alkylene glycol with, for example, a weight average molecular weight of from about 100 to about 20,000, from about 400 to about 5,000, or from about 1,000 to about 2,000, a charge transport compound; an acid catalyst, and a crosslinking agent wherein the overcoating layer, which is crosslinked, contains polyols, such as an acrylated polyol and a glycol, a crosslinking agent residue and a catalyst residue, all reacted into a polymeric network. While the percentage of crosslinking can be difficult to determine and not be desired to be limited by theory, the overcoat layer is crosslinked to a suitable value, such as for example, from about 5 to about 50 percent, from about 5 to about 25 percent, from about 10 to about 20 percent, and in embodiments from about 40 to about 65 percent. Excellent photoconductor electrical response can also be achieved when the prepolymer hydroxyl groups, and the hydroxyl groups of the dihydroxy aryl amine (DHTPD) are stoichiometrically less than the available methoxy alkyl on the crosslinking, such as CYMEL® moieties.

The photoreceptor overcoat can be applied by a number of different processes inclusive of dispersing the overcoat composition in a solvent system, and applying the resulting overcoat coating solution onto the receiving surface, for example, the top charge transport layer of the photoreceptor to a thickness of, for example, from about 0.5 micron to about 10, or from 0.5 to about 8 microns.

According to various embodiments, the crosslinkable polymer present in the overcoat layer can comprise a mixture of a polyol and acrylated polyol film forming resins, and where, for example, the crosslinkable polymer can be electrically insulating, semiconductive or conductive, and can be charge transporting or free of charge transporting characteristics. Examples of polyols include a highly branched polyol where highly branched refers, for example, to a prepolymer synthesized using a sufficient amount of trifunctional alcohols, such as triols or a polyfunctional polyol with a high hydroxyl number to form a polymer comprising a number of branches off of the main polymer chain. The polyol can possess a hydroxyl number of, for example, from about 10 to about 10,000 and can include ether groups, or can be free of ether groups. Suitable acrylated polyols can be, for example, generated from the reaction products of propylene oxide

31

modified with ethylene oxide, glycols, triglycerol and the like, and wherein the acrylated polyols in embodiments can be represented by



where  $R_s$  represents  $CH_2CR_1CO_2-$ ; where  $t=0$  to 1 and represents the mole fraction acrylic groups on available sites; where  $[R_s-CH_2]_t$  can be located in linear or branched portions of  $R_a$ ,  $R_b$ ,  $R_c$ , and  $R_d$ ;  $R_1$  is alkyl with, for example, from 1 to about 25 carbon atoms, and more specifically, from 1 to about 12 carbon atoms, such as methyl, ethyl, propyl, butyl, hexyl, heptyl, and the like;  $R_a$  and  $R_c$  independently represent linear alkyl groups, alkoxy groups, branched alkyl or branched alkoxy groups with alkyl and alkoxy groups possessing, for example, from 1 to about 20 carbon atoms;  $R_b$  and  $R_d$  independently represent alkyl or alkoxy groups having, for example, from 1 to about 20 carbon atoms; and  $m$ ,  $n$ ,  $p$ , and  $q$  represent mole fractions of from 0 to 1, such that  $n+m+p+q=1$ . Examples of commercial acrylated polyols are JONCRYL™ polymers, available from Johnson Polymers Inc. and POLYCHEM™ polymers, available from OPC polymers.

The overcoat layer includes in embodiments a crosslinking agent and catalyst where the crosslinking agent can be, for example, a melamine crosslinking agent or accelerator. Incorporation of a crosslinking agent can provide reaction sites to interact with the acrylated polyol to provide a branched, crosslinked structure. When so incorporated, any suitable crosslinking agent or accelerator can be used, including, for example, trioxane, melamine compounds, and mixtures thereof. When melamine compounds are selected, they can be functionalized, examples of which are melamine formaldehyde, methoxymethylated melamine compounds, such as glycouril-formaldehyde and benzoguanamine-formaldehyde, and the like. In some embodiments, the crosslinking agent can include a methylated, butylated melamine-formaldehyde. A nonlimiting example of a suitable methoxymethylated melamine compound can be CYMEL® 303 (available from Cytec Industries), which is a methoxymethylated melamine compound with the formula  $(CH_3OCH_2)_6N_3C_3N_3$  and the following structure



Crosslinking can be accomplished by heating the overcoating components in the presence of a catalyst. Non-limiting examples of catalysts include oxalic acid, maleic acid, carbolic acid, ascorbic acid, malonic acid, succinic acid, tartaric acid, citric acid, p-toluenesulfonic acid, methanesulfonic acid, and the like, and mixtures thereof.

A blocking agent can also be included in the overcoat layer, which agent can "tie up" or substantially block the acid catalyst effect to provide solution stability until the acid catalyst function is desired. Thus, for example, the blocking agent can block the acid effect until the solution temperature is raised above a threshold temperature. For example, some blocking

32

agents can be used to block the acid effect until the solution temperature is raised above about 100° C. At that time, the blocking agent dissociates from the acid and vaporizes. The unassociated acid is then free to catalyze the polymerization.

unassociated acid is then free to catalyze the polymerization.

5 Examples of such suitable blocking agents include, but are not limited to, pyridine and commercial acid solutions containing blocking agents such as CYCATE® 4045, available from Cytec Industries Inc.

The temperature used for crosslinking varies with the specific catalyst, the catalyst amount, heating time utilized, and the degree of crosslinking desired. Generally, the degree of crosslinking selected depends upon the desired flexibility of the final photoreceptor. For example, complete crosslinking, that is 100 percent, may be used for rigid drum or plate photoreceptors. However, partial crosslinking, for example, from about 20 percent to about 80 percent, is usually selected for flexible photoreceptors having, for example, web or belt configurations. The amount of catalyst to achieve a desired degree of crosslinking will vary depending upon the specific coating solution materials, such as polyol/acrylated polyol, catalyst, temperature, and time used for the reaction. Specifically, the polyester polyol/acrylated polyol is crosslinked at a temperature between about 100° C. and about 150° C. A typical crosslinking temperature used for polyols/acrylated polyols with p-toluenesulfonic acid as a catalyst is less than about 140° C., for example 135° C. for about 1 minute to about 40 minutes. A typical concentration of acid catalyst is from about 0.01 to about 5 weight percent based on the weight of polyol/acrylated polyol. After crosslinking, the overcoating should be substantially insoluble in the solvent in which it was soluble prior to crosslinking, thus permitting no overcoating material to be removed when rubbed with a cloth soaked in the solvent. Crosslinking results in the development of a three dimensional network which restrains the transport molecule in the crosslinked polymer network.

The overcoat layer can also include a charge transport material to, for example, improve the charge transport mobility of the overcoat layer. According to various embodiments, the charge transport material can be selected from the group 40 consisting of at least one of (i) a phenolic substituted aromatic amine, (ii) a primary alcohol substituted aromatic amine, and (iii) mixtures thereof. In embodiments, the charge transport material can be a terphenyl of, for example, an alcohol soluble dihydroxy terphenyl diamine; an alcohol-soluble dihydroxy 45 TPD, and the like. An example of a terphenyl charge transporting molecule can be represented by the following formula:



where each  $R_1$  is  $-\text{OH}$ ; and  $R_2$  is alkyl ( $-\text{C}_n\text{H}_{2n+1}$ ) where, for example,  $n$  is from 1 to about 10, from 1 to about 5, or from about 1 to about 6; and aralkyl and aryl groups with, for example, from about 6 to about 30, or about 6 to about 20 carbon atoms. Suitable examples of aralkyl groups include, for example,  $-\text{C}_n\text{H}_{2n}$ -phenyl groups where  $n$  is, for example, from about 1 to about 5 or from about 1 to about 10. Suitable examples of aryl groups include, for example, phenyl, naphthyl, biphenyl, and the like. In one embodiment, each  $R_1$  is

—OH to provide a dihydroxy terphenyl diamine hole transporting molecule. For example, where each R<sub>1</sub> is —OH and each R<sub>2</sub> is —H, the resultant compound is N,N'-diphenyl-N,N'-di[3-hydroxyphenyl]-terphenyl-diamine. In another embodiment, each R<sub>1</sub> is —OH, and each R<sub>2</sub> is independently an alkyl, aralkyl, or aryl group as defined above. In various embodiments, the charge transport material is soluble in the selected solvent used in forming the overcoat layer.

Any suitable secondary or tertiary alcohol solvent can be employed for the deposition of the film forming overcoat layer. Typical alcohol solvents include, but are not limited to, for example, tert-butanol, sec-butanol, 2-propanol, 1-methoxy-2-propanol, and the like, and mixtures thereof. Other suitable co-solvents that can be selected for the forming of the overcoat layer such as, for example, tetrahydrofuran, monochlorobenzene, and mixtures thereof. These co-solvents can be used as diluents for the above alcohol solvents, or they can be omitted. However, in some embodiments, it may be of value to minimize or avoid the use of higher boiling alcohol solvents since they should be removed as they may interfere with efficient crosslinking.

In embodiments, the components, including the crosslinkable polymer, charge transport material, crosslinking agent, acid catalyst, and blocking agent, utilized for the overcoat solution should be soluble or substantially soluble in the solvents or solvents employed for the overcoating.

The thickness of the overcoat layer, which can depend upon the abrasiveness of the charging (for example bias charging roll), cleaning (for example blade or web), development (for example brush), transfer (for example bias transfer roll), etc., in the system employed, is for example, from about 1 or about 2 microns up to about 10 or about 15 microns, or more. In various embodiments, the thickness of the overcoat layer can be from about 1 micrometer to about 5 micrometers. Typical application techniques for applying the overcoat layer over the photoconductive layer can include spraying, dip coating, roll coating, wire wound rod coating, and the like. Drying of the deposited overcoat layer can be effected by any suitable conventional technique such as oven drying, infrared radiation drying, air drying, and the like. The dried overcoat layer of this disclosure should transport charges during imaging.

In the dried overcoat layer, the composition can include from about 40 to about 90 percent by weight of film forming crosslinkable polymer, and from about 60 to about 10 percent by weight of charge transport material. For example, in embodiments, the charge transport material can be incorporated into the overcoat layer in an amount of from about 20 to about 50 percent by weight. As desired, the overcoat layer can also include other materials, such as conductive fillers, abrasion resistant fillers, and the like, in any suitable and known amounts.

Although not desired to be limited by theory, the crosslinking agent can be located in the central region with the polymers like the acrylated polyol, polyalkylene glycol, and also charge transport component being associated with the crosslinking agent, and extending in embodiments from the central region. Examples of components or materials optionally incorporated into the charge transport layers or at least one charge transport layer to, for example, enable improved lateral charge migration (LCM) resistance include hindered phenolic antioxidants, such as tetrakis methylene(3,5-di-tert-butyl-4-hydroxy hydrocinnamate) methane (IRGANOX® 1010, available from Ciba Specialty Chemical), butylated hydroxytoluene (BHT), and other hindered phenolic antioxidants including SUMILIZER™ BHT-R, MDP-S, BBM-S, WX-R, NW, BP-76, BP-101, GA-80, GM and GS (available

from Sumitomo Chemical Company, Ltd.), IRGANOX® 1035, 1076, 1098, 1135, 1141, 1222, 1330, 1425WL, 1520L, 245, 259, 3114, 3790, 5057 and 565 (available from Ciba Specialties Chemicals), and ADEKA STAB™ AO-20, 5 AO-30, AO-40, AO-50, AO-60, AO-70, AO-80 and AO-330 (available from Asahi Denka Company, Ltd.); hindered amine antioxidants such as SANOL™ LS-2626, LS-765, LS-770 and LS-744 (available from SNKYO CO., Ltd.), TINUVIN® 144 and 622LD (available from Ciba Specialties 10 Chemicals), MARK™ LA57, LA67, LA62, LA68 and LA63 (available from Asahi Denka Co., Ltd.), and SUMILIZER™ TPS (available from Sumitomo Chemical Co., Ltd.); thioether antioxidants such as SUMILIZER™ TP-D (available from Sumitomo Chemical Co., Ltd.); phosphite antioxidants such as MARK™ 2112, PEP-8, PEP-24G, PEP-36, 329K and 15 HP-10 (available from Asahi Denka Co., Ltd.); other molecules, such as bis(4-diethylamino-2-methylphenyl)phenylmethane (BDETPM), bis-[2-methyl-4-(N-2-hydroxyethyl-N-ethyl-aminophenyl)]-phenylmethane (DHTPM), and the 20 like. The weight percent of the antioxidant in at least one of the charge transport layers is from about 0 to about 20, from about 1 to about 10, or from about 3 to about 8 weight percent.

At least one charge transport layer refers, for example, to a single layer or a plurality of layers, such as from 1 to about 10 layers or more in certain situations, and more specifically, from 1 to about 4 layers, and yet more specifically 2 layers, and where one of the charge transport layers contains a thiophosphate, two charge transport layers contain a thiophosphate, 3, 4, or 5 charge transport layers contain a thiophosphate and in embodiments where a first charge transport layer 30 in contact with the photogenerating layer contains a thiophosphate and a second charge transport layer in contact with the first charge transport layer and in contact with the overcoating layer is free of a thiophosphate, and more specifically, polyethylene glycol, polypropylene glycol, polybutylene glycol, mixtures thereof, and the like.

Primarily for purposes of brevity, the examples of each of the substituents, and each of the components/compounds/molecules, polymers (components) for each of the layers 40 specifically disclosed herein are not intended to be exhaustive. Thus, a number of components, polymers, formulas, structures, and R group or substituent examples, and carbon chain lengths not specifically disclosed or claimed are intended to be encompassed by the present disclosure and claims. Also, the carbon chain lengths are intended to include all numbers between those disclosed or claimed or envisioned, thus from 1 to about 20 carbon atoms, and from 6 to about 36 carbon atoms includes 1, 2, 3, 4, 5, 6, 7, 8, 9, 10, 11, 12, 13, 14, 15, up to 36, or more. Similarly, the thickness of 45 each of the layers, the examples of components in each of the layers, the amount ranges of each of the components disclosed and claimed are not exhaustive, and it is intended that the present disclosure and claims encompass other suitable parameters not disclosed or that may be envisioned.

The following Examples are being submitted to illustrate embodiments of the present disclosure. These Examples are intended to be illustrative only, and are not intended to limit the scope of the present disclosure. Also, parts and percentages are by weight unless otherwise indicated. Comparative 50 Examples and data are also provided.

#### Comparative Example 1

An imaging member or photoconductor was prepared by 55 providing a 0.02 micrometer thick titanium layer coated (the coater device) on a biaxially oriented polyethylene naphthalate substrate (KALEDEX™ 2000) having a thickness of 3.5

mils, and applying thereon, with a gravure applicator, a solution containing 50 grams of 3-amino-propyltriethoxysilane, 41.2 grams of water, 15 grams of acetic acid, 684.8 grams of denatured alcohol, and 200 grams of heptane. This layer was then dried for about 5 minutes at 135° C. in the forced air dryer of the coater. The resulting blocking layer had a dry thickness of 500 Angstroms. An adhesive layer was then prepared by applying a wet coating over the blocking layer, using a gravure applicator, and which adhesive contains 0.2 percent by weight based on the total weight of the solution of copolyester adhesive (ARDEL D100<sup>TM</sup> available from Toyota Hsutsu Inc.) in a 60:30:10 volume ratio mixture of tetrahydrofuran/monochlorobenzene/methylene chloride. The adhesive layer was then dried for about 5 minutes at 135° C. in the forced air dryer of the coater. The resulting adhesive layer had a dry thickness of 200 Angstroms.

A photogenerating layer dispersion was prepared by introducing 0.45 grams of the known polycarbonate LUPILON 200<sup>TM</sup> (PCZ-200) or POLYCARBONATE Z<sup>TM</sup>, weight average molecular weight of 20,000, available from Mitsubishi Gas Chemical Corporation, and 44.65 grams of tetrahydrofuran into a 4 ounce glass bottle. To this solution were added 2.4 grams of hydroxygallium phthalocyanine (Type V) and 300 grams of  $\frac{1}{8}$  inch (3.2 millimeters) diameter stainless steel shot. This hydroxygallium phthalocyanine mixture was then placed on a ball mill at 200 RPM for 8 hours. Subsequently, 0.8 grams of PCZ-200 were dissolved in 12.86 grams of tetrahydrofuran, and added to 20 grams of the hydroxygallium phthalocyanine dispersion above. This slurry was then placed on a shaker for 15 minutes. The resulting dispersion was, thereafter, applied to the above adhesive interface with a Bird applicator to form a photogenerating layer having a wet thickness of 0.25 mil. A strip about 10 millimeters wide along one edge of the substrate web bearing the blocking layer, and the adhesive layer was deliberately left uncoated by any of the photogenerating layer material to facilitate adequate electrical contact by the ground strip layer that was applied later. The charge generation layer was dried at 135° C. for 5 minutes in a forced air oven to form a dry photogenerating layer having a thickness of 0.4 micrometer.

The resulting imaging member web was then overcoated with a two-layer charge transport layer. Specifically, the photogenerating layer was overcoated in a first pass with a charge transport layer (the bottom layer) in contact with the photogenerating layer. The bottom layer of the charge transport layer was prepared by introducing into an amber glass bottle in a weight ratio of 1:1 N,N'-diphenyl-N,N'-bis(3-methylphenyl)-1,1'-biphenyl-4,4'-diamine, and MAKROLON 5705<sup>®</sup>, a known polycarbonate resin having a molecular weight average of from about 50,000 to about 100,000, commercially available from Farbenfabriken Bayer A.G. The resulting mixture was then dissolved in methylene chloride to form a solution containing 15 percent by weight solids. This solution was applied on the photogenerating layer to form the bottom layer coating that upon drying (120° C. for 1 minute) had a thickness of 14.5 microns. During this coating process, the humidity was equal to or less than 15 percent.

The bottom layer of the charge transport layer (CTL) was then overcoated with a top charge transport layer in a second pass. The charge transport layer solution of the top layer was prepared by introducing into an amber glass bottle in a weight ratio of 1:1 N,N'-diphenyl-N,N'-bis(3-methylphenyl)-1,1'-biphenyl-4,4'-diamine, and MAKROLON 5705<sup>®</sup>, a known polycarbonate resin having a molecular weight average of from about 50,000 to about 100,000, commercially available from Farbenfabriken Bayer A.G. This solution was applied, using a 2 mil Bird bar, on the bottom layer of the charge

transport layer to form a coating that upon drying (120° C. for 1 minute) had a thickness of 14.5 microns. Total CTL thickness was 29 microns.

#### Example II

##### Preparation of Overcoat Coating Solution

An overcoat coating solution was formed by adding 10 grams of POLYCHEM<sup>®</sup> 7558-B-60 (an acrylated polyol obtained from OPC Polymers), 4 grams of PPG 2K (a polypropylene glycol with a weight average molecular weight of 2,000 as obtained from Sigma-Aldrich), 6 grams of CYMEL<sup>®</sup> 1130 (a methylated, butylated melamine-formaldehyde crosslinking agent obtained from Cytec Industries Inc.), 8 grams of N,N'-diphenyl-N,N'-di[3-hydroxyphenyl]-terphenyl-diamine (DHTPD), 1.5 grams of SILCLEAN<sup>™</sup> 3700 (a hydroxylated silicone available from BYK-Chemie USA), and 5.5 grams [1 percent by weight] of 8 percent p-toluenesulfonic acid catalyst in 60 grams of DOWANOL<sup>®</sup> PM (1-methoxy-2-propanol obtained from the Dow Chemical Company).

#### Comparative Example 3

The photoreceptor device of Comparative Example 1 was overcoated with the solution of Example II using a  $\frac{1}{8}$  mil Bird bar. The resultant film was dried in a forced air oven for 2 minutes at 125° C. to yield a highly crosslinked, 3 micron overcoat in contact with the top CTL, and which overcoat was substantially insoluble in methanol or ethanol.

#### Example IV

An imaging member was prepared by essentially repeating the process of Comparative Example 1 except that to the photogenerating layer dispersion of Comparative Example 1 were added 0.06 grams of zinc dialkyldithiophosphate (ZDDP ELCO-103<sup>TM</sup>, wherein alkyl is a mixture of primary butyl and primary octyl), commercially available from Elco Corporation.

The resulting dispersion was, thereafter, applied to the above adhesive interface with a Bird applicator to form a photogenerating layer having a wet thickness of 0.25 mil. The charge generation layer was dried at 135° C. for 5 minutes in a forced air oven to form a dry photogenerating layer having a thickness of 0.4 micrometer. The bottom layer of the charge transport layer was prepared by introducing into an amber glass bottle in a weight ratio of 46:46:8 N,N'-diphenyl-N,N'-bis(3-methylphenyl)-1,1'-biphenyl-4,4'-diamine, MAKROLON<sup>®</sup> 5705, a polycarbonate resin having a weight average molecular weight of from about 50,000 to about 100,000, commercially available from Farbenfabriken Bayer A.G., and phenyl-POSS trisilanol (SO1458<sup>TM</sup>, available from Hybrid Plastics, Fountain Valley, Calif.). The resulting mixture was dissolved in methylene chloride to form a solution containing 15 percent by weight solids. This solution was applied, using a 2 mil Bird bar, on the photogenerating layer to form the bottom layer coating that upon drying (120° C. for 1 minute) had a thickness of 14.5 microns.

The bottom layer of the charge transport layer was then overcoated with a top layer. The charge transport layer solution of the top layer was prepared by introducing into an amber glass bottle in a weight ratio of 1:1 N,N'-diphenyl-N,N'-bis(3-methylphenyl)-1,1'-biphenyl-4,4'-diamine, and MAKROLON<sup>®</sup> 5705, a known polycarbonate resin having a molecular weight average of from about 50,000 to about 100,000 to about

100,000, commercially available from Farbenfabriken Bayer A.G. This solution was applied on the bottom layer of the charge transport layer, using a 2 mil Bird bar, to form a coating that upon drying (120° C. for 1 minute) had a thickness of 14.5 microns. During this coating process, the humidity was equal to or less than 15 percent. The total CTL (bottom and top charge transport layer) thickness was 29 microns.

#### Example V

The photoreceptor device of Example IV was overcoated with the solution of Example II using a  $\frac{1}{8}$  mil Bird bar. The resultant film was dried in a forced air oven for 2 minutes at 125° C. to yield a highly crosslinked, 3 micron overcoat, and which overcoat was substantially insoluble in methanol or ethanol.

#### Example VI

An imaging member was prepared by repeating the process of Comparative Example 1 except that to the photogenerating layer dispersion of Comparative Example 1 were added 0.12 grams of the above zinc dialkyldithiophosphate (ZDDP ELCO-103™, wherein alkyl is a mixture of primary butyl and primary octyl), commercially available from Elco Corporation.

The resulting dispersion was, thereafter, applied to the above adhesive interface with a Bird applicator to form a photogenerating layer having a wet thickness of 0.25 mil. The charge generation layer was dried at 135° C. for 5 minutes in a forced air oven to form a dry photogenerating layer having a thickness of 0.4 micrometer. The bottom layer of the charge transport layer was prepared by introducing into an amber glass bottle in a weight ratio of 46:46:8 N,N'-diphenyl-N,N'-bis(3-methylphenyl)-1,1'-biphenyl-4,4'-diamine, MAKROLON® 5705, a polycarbonate resin having a weight average molecular weight of from about 50,000 to about 100,000, commercially available from Farbenfabriken Bayer A.G., and phenyl-POSS trisilanol (SO1458™, available from Hybrid Plastics, Fountain Valley, Calif.). The resulting mixture was dissolved in methylene chloride to form a solution containing 15 percent by weight solids. This solution was applied, using a 2 mil Bird bar, on the photogenerating layer to form the bottom layer coating that upon drying (120° C. for 1 minute) had a thickness of 14.5 microns.

The bottom layer of the charge transport layer was then overcoated with a top layer. The charge transport layer solution of the top layer was prepared by introducing into an amber glass bottle in a weight ratio of 1:1 N,N'-diphenyl-N,N'-bis(3-methylphenyl)-1,1'-biphenyl-4,4'-diamine, and MAKROLON® 5705, a known polycarbonate resin having a molecular weight average of from about 50,000 to about 100,000, commercially available from Farbenfabriken Bayer A.G. This solution was applied on the bottom layer of the charge transport layer, using a 2 mil Bird bar, to form a coating that upon drying (120° C. for 1 minute) had a thickness of 14.5 microns. During this coating process, the humidity was equal to or less than 15 percent. The total CTL (bottom and top charge transport layer) thickness was 29 microns.

#### Example VII

The photoconductor of Example VI was overcoated with the solution from Example VI using a  $\frac{1}{8}$  mil Bird bar. The resultant film was dried in a forced air oven for 2 minutes at 125° C. to yield a highly crosslinked, 3 micron overcoat, and which overcoat was substantially insoluble in methanol or ethanol.

#### Example VIII

#### Electrical Property Testing

5 A number of the above prepared photoconductors were tested in a scanner set to obtain photoinduced discharge cycles, sequenced at one charge-erase cycle followed by one charge-expose-erase cycle, wherein the light intensity was incrementally increased with cycling to produce a series of photoinduced discharge characteristic (PIDC) curves from which the photosensitivity and surface potentials at various exposure intensities were measured. Additional electrical characteristics were obtained by a series of charge-erase cycles with incrementing surface potential to generate several voltage versus charge density curves. The scanner was equipped with a scorotron set to a constant voltage charging at various surface potentials. The devices were tested at surface potentials of 500 with the exposure light intensity incrementally increased by means of regulating a series of neutral density filters; the exposure light source is a 780 nanometer light emitting diode. A xerographic simulation was completed in an environmentally controlled light tight chamber at ambient conditions (40 percent relative humidity and 22° C.).

10 15 20 25 30

20 25 30

35 40

45 50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4875

4880

4885

4890

4895

4900

4905

4910

4915

4920

4925

4930

4935

4940

4945

4950

4955

4960

4965

4970

4975

4980

4985

4990

4995

5000

5005

5010

5015

5020

5025

5030

5035

5040

5045

5050

5055

5060

5065

5070

5075

5080

5085

5090

5095

5100

5105

5110

5115

5120

5125

5130

5135

5140

5145

5150

5155

5160

5165

5170

5175

5180

5185

5190

5195

5200

5205

5210

5215

5220

5225

5230

5235

5240

5245

5250

5255

5260

5265

5270

5275

5280

5285

5290

5295

5300

5305

5310

5315

5320

5325

5330

5335

5340

5345

5350

5355

5360

5365

5370

5375

5380

5385

5390

5395

5400

5405

5410

5415

5420

5425

5430

5435

5440

5445

5450

5455

5460

5465

5470

5475

5480

5485

5490

5495

5500

5505

5510

5515

5520

5525

5530

5535

5540

5545

5550

5555

5560

What is claimed is:

1. An imaging member comprising an optional supporting substrate, a photogenerating layer, and at least one charge transport layer, and wherein said photogenerating layer contains at least one thiophosphate, and an overcoating layer in contact with and contiguous to said charge transport layer, and which overcoating is comprised of an acrylated polyol, a polyalkylene glycol, a crosslinking component, and a charge transport component.

2. An imaging member in accordance with claim 1 wherein said photogenerating layer is comprised of at least one photogenerating pigment and said thiophosphate; and wherein said overcoating is generated in the presence of a catalyst by the reaction of said polyol, said glycol, said crosslinking component, and said charge transport component to form a polymer network.

3. An imaging member in accordance with claim 1 wherein said photogenerating layer is comprised of a photogenerating component, a polymer binder, and said at least one thiophosphate.

4. An imaging member in accordance with claim 1 wherein said charge transport layer is comprised of aryl amine molecules, and which aryl amines are of the formula



wherein X is selected from the group consisting of alkyl, alkoxy, aryl, and halogen, and mixtures thereof.

5. An imaging member in accordance with claim 4 wherein each of said alkoxy and alkyl contain from about 1 to about 10 carbon atoms, and said X substituent is present on each of the four terminal rings.

6. An imaging member in accordance with claim 4 wherein said aryl amine is N,N'-diphenyl-N,N-bis(3-methylphenyl)-1,1'-biphenyl-4,4'-diamine.

7. An imaging member in accordance with claim 1 wherein said charge transport layer is comprised of



wherein each X and Y is independently selected from the group consisting of at least one of alkyl, alkoxy, aryl, and halogen.

8. An imaging member in accordance with claim 7 wherein each alkoxy and alkyl contains from about 1 to about 10 carbon atoms; aryl contains from 6 to about 36 carbon atoms; and halogen is chloride, bromide, fluoride, or iodide.

9. An imaging member in accordance with claim 1 wherein said charge transport layer contains a component selected

from the group consisting of N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis-(4-isopropylphenyl)-[p-terphenyl]-4,4"-diamine, N,N'-bis(4-butylphenyl)-N,N'-bis-(2-ethyl-6-methylphenyl)-[p-terphenyl]-4,4"-diamine, N,N'-bis(4-butylphenyl)-N,N'-bis-(2,5-dimethylphenyl)-[p-terphenyl]-4,4"-diamine, and N,N'-diphenyl-N,N'-bis(3-chlorophenyl)-[p-terphenyl]-4,4"-diamine, and optionally mixtures thereof.

10. An imaging member in accordance with claim 1 wherein said at least one charge transport layer contains an antioxidant comprised of a hindered phenol or a hindered amine.

15. An imaging member in accordance with claim 1 wherein said at least one charge transport layer is from 1 to about 7 layers; said at least one thiophosphate is from 1 to about 3; and said alkylene contains from 2 to about 14 carbon atoms.

20. An imaging member in accordance with claim 1 wherein said at least one charge transport layer is from 1 to about 3 layers.

25. An imaging member in accordance with claim 1 wherein said at least one charge transport layer is comprised of a top charge transport layer and a bottom charge transport layer, and wherein said bottom layer is situated between said photogenerating layer and said top charge transport layer.

30. An imaging member in accordance with claim 1 wherein said top layer is comprised of at least one charge transport component and at least one polymer binder, and said bottom layer is comprised of at least one charge transport component and at least one resin binder; wherein said glycol is a polypropylene glycol; and said overcoating is generated in the presence of a catalyst by the reaction of said polyol, said glycol, said crosslinking component, and said charge transport component to form a polymer network.

35. An imaging member in accordance with claim 1 wherein said thiophosphate is a zinc dialkyldithiophosphate.

40. An imaging member in accordance with claim 1 wherein said photogenerating layer is coated from a photogenerating dispersion prepared by adding said thiophosphate into a dispersion of a photogenerating layer component, and a polymeric resin, or by ball milling said thiophosphate, a photogenerating layer component, and a polymeric resin.

45. An imaging member in accordance with claim 1 wherein said photogenerating layer is comprised of at least one of a metal phthalocyanine, metal free phthalocyanine, titanyl phthalocyanine, a halogallium phthalocyanine, a perylene, or mixtures thereof.

50. An imaging member in accordance with claim 1 wherein said photogenerating layer is comprised of a chlorogallium phthalocyanine pigment, or a hydroxygallium phthalocyanine.

55. An imaging member in accordance with claim 1 wherein said thiophosphate is metal free or metal containing thiophosphate, and wherein said metal is selected from the group consisting of zinc, molybdenum, lead, manganese, and antimony, and mixtures thereof.

41

20. An imaging member in accordance with claim 1 wherein said thiophosphate is



wherein R<sub>1</sub>, R<sub>2</sub>, R<sub>3</sub>, R<sub>4</sub>, R<sub>5</sub> and R<sub>6</sub> each independently represents a hydrogen atom, alkyl, cycloalkyl, aryl, alkylaryl, arylalkyl or mixtures thereof.

21. An imaging member in accordance with claim 20 wherein R<sub>1</sub>, R<sub>2</sub>, R<sub>3</sub>, R<sub>4</sub>, R<sub>5</sub> and R<sub>6</sub> each independently represents alkyl containing from 1 to about 20 carbon atoms; cycloalkyl containing from 6 to about 26 carbon atoms; aryl, alkylaryl or arylalkyl containing from about 6 to about 50 carbon atoms; or optionally a hydrocarbyl group.

22. An imaging member in accordance with claim 1 wherein said thiophosphate is a zinc dialkyldithiophosphate, and wherein said alkyl is a straight chain or branched alkyl with from about 2 to about 18 carbon atoms.

23. An imaging member in accordance with claim 1 wherein said thiophosphate is present in an amount of from about 0.1 to about 40 weight percent.

24. An imaging member in accordance with claim 1 wherein said thiophosphate is present in an amount of from about 0.5 to about 15.

25. An imaging member in accordance with claim 1 wherein at least one photogenerating layer is one, wherein at least one thiophosphate is from 1 to about 3, and wherein said thiophosphate is present in an amount of from about 1 to about 10 weight percent.

26. An imaging member in accordance with claim 1 wherein said acrylated polyol is represented by



where R<sub>s</sub> represents CH<sub>2</sub>CR<sub>1</sub>CO<sub>2</sub>—; where t=0 to 1 and represents the mole fraction acrylic groups on available sites; where [R<sub>s</sub>—CH<sub>2</sub>]<sub>t</sub> can be located in linear or branched portions of R<sub>a</sub>, R<sub>b</sub>, R<sub>c</sub>, and R<sub>d</sub>; where R<sub>a</sub> and R<sub>c</sub> independently represent at least one of an alkyl group, an alkoxy group; R<sub>b</sub> and R<sub>d</sub> independently represent at least one of an alkyl and alkoxy; and m, n, p, and q represent mole fractions, such that n+m+p+q=1; and wherein said overcoating primarily contains said acrylate polyol, said glycol, said crosslinking agent, and said charge transport compound.

27. An imaging member in accordance with claim 1 wherein said at least one charge transport layer further contains a silanol.

28. A flexible photoconductive member comprised in sequence of a substrate, a photogenerating layer, and at least one charge transport layer comprised of at least one charge

42

transport component, and wherein said photogenerating layer is comprised of at least one photogenerating pigment, and the thiophosphate



wherein R<sub>1</sub>, R<sub>2</sub>, R<sub>3</sub>, R<sub>4</sub>, R<sub>5</sub> and R<sub>6</sub> each independently represents at least one of a hydrogen atom, and alkyl, aryl, cycloalkyl, and alkylaryl; and an overcoating in contact with and contiguous to said charge transport layer, and which overcoating is formed from an acrylate polyol, a polyalkylene glycol, a crosslinking agent, a charge transport compound, and a catalyst.

29. A member in accordance with claim 28 where at least one is one for said photogenerating layer; at least one is from 1 to about 3 for said charge transport layer; and at least one is one for said thiophosphate, and wherein said suitable hydrocarbon is alkyl, cycloalkyl, aryl, alkylaryl or arylalkyl.

30. An imaging member in accordance with claim 1 further including a hole blocking layer, and an adhesive layer.

31. An imaging member in accordance with claim 1 wherein said thiophosphate is molybdenum di(2-ethylhexyl) dithiophosphate, zinc diethyldithiophosphate, or antimony diamyldithiophosphate.

32. A member in accordance with claim 28 wherein said acrylated polyol is represented by



where R<sub>s</sub> represents CH<sub>2</sub>CR<sub>1</sub>CO<sub>2</sub>—; where t=0 to 1 and represents the mole fraction acrylic groups on available sites; where [R<sub>s</sub>—CH<sub>2</sub>]<sub>t</sub> can be located in linear or branched portions of R<sub>a</sub>, R<sub>b</sub>, R<sub>c</sub>, and R<sub>d</sub>; where R<sub>a</sub> and R<sub>c</sub> independently represent at least one of a linear alkyl group, a linear alkoxy group, a branched alkyl group, and a branched alkoxy group, wherein each alkyl and alkoxy group contain from about 1 to about 20 carbon atoms; R<sub>b</sub> and R<sub>d</sub> independently represent at least one of an alkyl and alkoxy wherein said alkyl and said alkoxy each contain from about 1 to about 20 carbon atoms; and m, n, p, and q represent mole fractions, such that n+m+p+q=1.

33. A member in accordance with claim 28 wherein said at least one charge transport layer further contains a silanol.

34. A photoconductor comprising a supporting substrate, a photogenerating layer, at least one charge transport layer, and wherein said photogenerating layer is comprised of at least one photogenerating pigment, and a dialkyldithiophosphate encompassed by



wherein R<sub>1</sub>, R<sub>2</sub>, R<sub>3</sub>, R<sub>4</sub>, R<sub>5</sub> and R<sub>6</sub> each independently represents a hydrogen atom, alkyl and aryl, or mixtures thereof;

20

and wherein said photogenerating layer and said charge transport layer include a resin binder; wherein said at least one charge transport layer is from 2 to about 5, and said photogenerating layer is situated between said substrate and said at least one charge transport; and a layer in contact with and contiguous to the top charge transport layer, and which layer is comprised of a crosslinked polymeric network.

35. A photoconductor in accordance with claim 34 wherein the dialkyldithiophosphate is zinc diethyldithiophosphate, 10 and at least one charge transport is comprised of a first charge transport layer in contact with the photogenerating layer and a second charge transport layer thereover in contact with the overcoating generated in the presence of a catalyst by the reaction of said polyol, said glycol, said crosslinking component, and said charge transport component to form a polymer network.

36. A photoconductor in accordance with claim 34 wherein said at least one charge transport layer further contains a silanol.

\* \* \* \* \*